

United States Patent [19]  
Millikan et al.

[11] 3,753,721  
[45] Aug. 21, 1973

[54] PHOTOGRAPHIC MATERIALS

[75] Inventors: Allan G. Millikan, Webster; Mary Jane W. Brizee, Pittsford, both of N.Y.

[73] Assignee: Eastman Kodak Company, Rochester, N.Y.

[22] Filed: Aug. 13, 1970

[21] Appl. No.: 63,606

[52] U.S. Cl..... 96/130, 96/127, 96/108

[51] Int. Cl..... G03c 1/28

[58] Field of Search..... 96/108, 127, 130

[56] References Cited

UNITED STATES PATENTS

|           |       |                  |        |
|-----------|-------|------------------|--------|
| 2,839,403 | /1958 | Knott.....       | 96/127 |
| 3,573,920 | /1971 | Hiller.....      | 96/130 |
| 2,597,856 | /1952 | Damschroder..... | 96/108 |

|           |       |                         |        |
|-----------|-------|-------------------------|--------|
| 2,642,361 | /1953 | Damschroder et al. .... | 96/108 |
| 2,448,060 | /1948 | Smith et al. ....       | 96/108 |
| 2,540,085 | /1951 | Baldsiefen. ....        | 96/108 |

Primary Examiner—Ronald H. Smith

Assistant Examiner—Edward C. Kimlin

Attorney—W. H. J. Kline, J. R. Frederick and O. H. Webster

[57] ABSTRACT

Light-sensitive silver halide grains having an average size of up to 0.2 micron are sensitized with a noble metal sensitizer at a concentration of at least 50 mg. noble metal per mole of silver, and a sulfur sensitizer at a weight ratio of sulfur to noble metal of about 1:15 to 1:75; said silver halide grains being spectrally sensitized with a photographic spectral sensitizing methine dye.

20 Claims, No Drawings

## PHOTOGRAPHIC MATERIALS

This invention relates to photographic materials, and more particularly to fine grain silver halide photographic materials.

The combination of noble metal sensitizers and sulfur sensitizers has been suggested in the prior art for photographic silver halide emulsions. Typical disclosures of such sensitizers are made by Smith et al. in U.S. Pat. No. 2,448,060 issued Aug. 31, 1948, Baldsiefen U.S. Pat. No. 2,540,085 issued Feb. 6, 1951; Damschroder U.S. Pat. No. 2,597,856 issued May 27, 1952 and Damschroder et al. U.S. Pat. No. 2,642,361 issued June 16, 1953. Hiller in U.S. Pat. application Ser. No. 757,789 filed Sept. 5, 1968 now U.S. Pat. No. 3,573,920, and corresponding to Belgian Pat. No. 724,740 of Dec. 31, 1969, describes spectrally sensitized fine grain silver halide emulsions and states that such emulsions can be sensitized with sulfur and gold sensitizers. However, none of these references, nor any other reference known to applicants, suggest the sensitization of fine grain silver halide emulsions with a high concentration of noble metal sensitizer together with a low concentration of sulfur sensitizer.

Previously, it had been assumed that noble metal sensitization was most effective with large silver halide grains. Glafkides, *Photographic Chemistry*, published by the Fountain Press, London, 1958, states at page 320 that gold sensitization is mainly effective with large silver halide grains, which have higher sensitivity to light than fine silver halide grains (i.e., up to 0.2 micron in size). Glafkides also states at page 319 that gold sensitization frequently results in substantial increases in fog and causes emulsion instability, which often results in the emulsion becoming useless after being kept for a few days.

Fine grain silver halide emulsions must be used instead of faster large grain silver halide emulsions for various purposes, for example in photographic applications where high resolution is essential, such as holography and microphotography. Hence, it appears highly desirable to provide stable emulsions comprising fine silver halide grains which have low fog and high speeds.

One object of this invention is to provide photographic silver halide grains which exhibit increased speed to blue radiation.

Another object of this invention is to provide chemically sensitized photographic silver halide emulsions which are stable and exhibit increased speed to blue radiation.

A further object of this invention is to provide photographic silver halide emulsions which are particularly useful in applications requiring high resolving power, such as holography and microphotography.

Still another object of this invention is to provide spectrally sensitized photographic silver halide emulsions.

Another object of this invention is to provide spectrally sensitized fine grain silver halide emulsions having higher speeds in the region of spectral sensitivity.

Other objects of this invention will be apparent from this disclosure and the appended claims.

In accordance with this invention, light-sensitive silver halide grains having an average grain size up to about 0.2 micron are sensitized with the combination of a noble metal sensitizer, at a concentration of about at least 50 milligrams noble metal per mole of silver,

and a sulfur sensitizer at a weight ratio of sulfur to noble metal of about 1:15 to 1:75; and, the silver halide grains are spectrally sensitized with a photographic spectral sensitizing methine dye.

The combination of a high concentration of noble metal sensitizer and a low concentration of sulfur sensitizer, together with a photographic spectral sensitizing dye, results in substantial and unexpected speed increases in the region of inherent sensitivity of silver halide grains. The increase in inherent sensitivity is accomplished without causing high fog or emulsion instability.

Silver halide grains employed in the practice of this invention can comprise silver chloride, silver bromide, silver bromoiodide, silver chlorobromoiodide or mixtures thereof. The silver halide grains can range in size up to 0.2 micron, and preferably up to 0.15 or 0.1  $\mu\text{m}$ . Grains in the range of about 0.02 up to 0.09 micron give excellent results. Such silver halide grains can be prepared by any of the well-known procedures. Very fine grain emulsions known in the art as "Lippmann" emulsions are useful herein.

The noble metal sensitizers useful in this invention include the well-known gold sensitizers and other noble metals such as palladium and platinum, including any of the noble metal sensitizers described in Smith et al U.S. Pat. No. 2,448,060 issued Aug. 31, 1948. Typical useful gold sensitizers are described in Waller et al U.S. Pat. No. 2,399,083 issued Apr. 23, 1946, Baldesiefen U.S. Pat. Nos. 2,540,085 and 2,540,086 both issued Feb. 6, 1951; Damschroder U.S. Pat. No. 2,597,856 issued May 27, 1952 and Damschroder et al. U.S. Pat. No. 2,642,361 issued June 16, 1953. Illustrative addenda suitable for furnishing the noble metal moiety in accordance with this invention include:

gold chloride potassium aurate,

potassium auraurite,

potassium auricyanide,

potassium aurithiocyanate,

gold sulfide,

gold selenide,

gold iodide,

potassium chloroaurate,

ethylenediamine-bis-gold chloride,

ammonium chloropalladate, i.e.,  $(\text{NH}_4)_2\text{PtCl}_6$ ,

ammonium chloropalladate, i.e.,  $(\text{NH}_4)_2\text{PdCl}_6$ , and

organic gold sensitizers having the formulas:





S-S-C- group. Typical sulfur sensitizers are thiourea, allylisothiocyanate, thiosinamine (allylthiourea), cystine and  $\beta$ -ethyl xanthate propionic acid. Also useful are methyl or ammonium thiocyanates, such as alkali metal thiocyanates (e.g., sodium or potassium thiocyanate) or alkaline earth metal thiocyanates (e.g., calcium thiocyanine, strontium thiocyanate, etc.), cadmium thiocyanate and ammonium thiocyanate. Especially useful are the alkali metal thiosulfates, preferably sodium or potassium thiosulfate, or ammonium thiosulfate. Thioureas, such as those referred to above, also produce particularly useful results.

Sulfur sensitizers are employed herein at a weight ratio of sulfur to noble metal of about 1:15 to 1:75, and preferably about 1:30 to about 1:50. The amount of labile sulfur, not the entire weight of the compound containing the labile sulfur, is used in calculating the useful concentrations of sulfur. As will be apparent to those skilled in the art, certain sulfur sensitizers (e.g., sodium thiosulfate) contain two sulfur atoms, but only one of those sulfur atoms is labile. These compounds are used in concentrations calculated on the basis of the one labile sulfur atom therein.

Any methine (including polymethine) photographic spectral sensitizing dye can be employed in the practice of this invention. The most useful methine dyes are the cyanine, merocyanine, hemicyanine and hemioxonol dyes. The dyes can be used in widely varying concentrations, with optimum concentrations being determined by any suitable means previously described in the art. Generally, about 100 to 2,000 mg. dye per mole of silver provide good results, although larger or smaller amounts produce useful results depending on the particular dye and silver halide used.

Typical useful cyanine dyes have the following general formula:



wherein  $d$  and  $n$  each represents a positive integer of from 1 to 2,  $m$  represents a positive integer of from 1 to 5, each  $L$  represents a methine group (e.g.,  $-CH=$ ,  $-C(CH_3)=$ , etc.), and  $Z$  and  $Z_1$  each represents the non-metallic atoms necessary to complete a heterocyclic nucleus containing from 5 to 6 atoms, such as used in cyanine dyes, which nuclei can contain a second hetero atom such as oxygen, sulfur, selenium or nitrogen, such as the following nuclei: a thiazole nucleus, e.g., thiazole, 4-methylthiazole, 4-phenylthiazole, 5-methylthiazole, 5-phenyl-thiazole, 4,5-dimethylthiazole, 4,5-diphenylthiazole, 4-(2-thienyl)thiazole, benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methyl-benzothiazole, 5-bromobenzothiazole, 6-bromobenzothiazole, 5-phenylbenzothiazole, 6-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxy benzothiazole, 5,6-dioxymethylenebenzothiazole, 5-hydroxy benzothiazole, 6-hydroxybenzothiazole, naphtho[2,1-d]thiazole, naph-

The noble metal sensitizer is employed in accordance with the invention in a concentration of from at least about 50 milligrams of noble metal per mole of silver, and preferably from about 125 to 175 milligrams noble metal sensitizer per mole of silver. Note that concentrations of noble metal are expressed in terms of noble metal and are not based on the total weight of the compound containing the noble metal. The noble metal sensitizer is employed at concentrations lower than which causes substantial fog, such as fog levels over 3. Generally, there is no advantage in employing over 200 mg. noble metal per mole of silver.

In accordance with the invention, the silver halide grains are chemically sensitized with a sulfur sensitizer. Sulfur sensitizers are well known in the art and are described, for example, by Damschroder et al. U.S. Pat. No. 2,642,361 issued June 16, 1953, columns 3 and 4. Typical sulfur sensitizers contain a  $=C=S$  group or a  $-C$

tho[1,2-d]thiazole, 5-methoxynaphtho[2,3-d]thiazole, 8-  
5-ethoxynaphtho[2,3-d]thiazole, 7-  
methoxynaphtho[2,3-d]thiazole, 4'-methoxythianaph-  
tho-7',6'-4,5-thiazole, etc.; an oxazole nucleus, e.g.,  
4-methyloxazole, 5-methyloxazole, 4-phenyloxazole,  
4,5-diphenyloxazole, 4-ethyloxazole, 4,5-  
dimethyloxazole, 5-phenyloxazole, benzoxazole, 5-  
chlorobenzoxazole, 5-methylbenzoxazole, 5-  
phenylbenzoxazole, 6-methylbenzoxazole, 5,6-dime-  
thylbenzoxazole, 4,6-dimethylbenzoxazole, 5-  
methoxybenzoxazole, 5-methoxybenzoxazole, 5-  
chlorobenzoxazole, 6-methoxybenzoxazole, 5-  
hydroxybenzoxazole, 6-hydroxybenzoxazole, naph-  
tho[2,1-d]oxazole, naphtho[1,2-d]oxazole, etc.; a  
selenazole nucleus, e.g., 4-methylselenazole, 4-  
phenylselenazole, benzoselenazole, 5-  
chlorobenzoselenazole, 5-methoxybenzoselenazole,  
5-hydroxybenzoselenazole, tetrahydro-  
benzoselenazole, naphtho[2,1-d]selenazole, naph-  
tho[1,2-d]selenazole, etc.; a thiazoline nucleus, e.g.,  
thiazoline, 4-methylthiazoline, etc.; a pyridine nucleus,  
e.g., 2-pyridine, 5-methyl-2-pyridine, 4-pyridine,  
3-methyl-4-pyridine, etc.; a quinoline nucleus, e.g., 2-  
quinoline, 3-methyl-2-quinoline, 5-ethyl-2-quinoline,  
6-chloro-2-quinoline, 8-chloro-2-quinoline, 6-methoxy-  
2-quinoline, 8-ethoxy-2-quinoline, 8-hydroxy-2-  
quinoline, 4-quinoline, 6-methoxy-4-quinoline,  
7-methyl-4-quinoline, 8-chloro-4-quinoline, 1-  
isoquinoline, 3,4-dihydro-1-isoquinoline, 3-  
isoquinoline, etc.; a 3,3-dialkylindolenine nucleus, e.g.,  
3,3-dimethylindolenine, 3,3,5-trimethylindolenine,  
etc.; and, an imidazole nucleus, e.g., imidazole, 1-  
alkylimidazole, 1-alkyl-4-phenylimidazole, 1-alkyl-4,5-  
dimethylimidazole, benzimidazole, 1-  
alkylbenzimidazole, 1-aryl-5,6-dichlorobenzimidazole,  
1-alkyl-1H-naphtho[1,2-d]imidazole, 1-aryl-3H-  
naphtho[1,2-d]imidazole, 1-alkyl-5-methoxy-1H-  
naphtho[1,2-d]imidazole, etc.; X represents an acid  
anion, such as chloride, bromide p-toluenesulfonate,  
methane sulfonate, methylsulfate, ethylsulfate, per-  
chlorate, etc.; R<sub>1</sub> and R<sub>2</sub> each represents an alkyl group  
(including substituted alkyl) having from 1 to 18, and  
preferably one to four carbon atoms, such as methyl,  
ethyl, propyl, isopropyl, butyl, sec-butyl, hexyl, dode-  
cyl, octadecyl, benzyl,  $\beta$ -phenylethyl, sulfoalkyl such as  
 $\beta$ -sulfoethyl,  $\gamma$ -sulfopropyl,  $\gamma$ -sulfobutyl,  $\delta$ -sulfobutyl,  
etc.; carboxyalkyl such as  $\beta$ -carboxyethyl,  $\gamma$ -carboxy-  
propyl,  $\delta$ -carboxybutyl, etc.; sulfatoalkyl such as  $\gamma$ -sul-  
foatopropyl and  $\delta$ -sulfatobutyl, etc. It will be noted that  
in some instances, the acid anion, represented by X in  
the above formula, is included in the substituent repre-  
sented by R<sub>2</sub>, such as dyes containing the betaine type  
structure. Some specific cyanine dyes that can be used  
in the process of this invention include the following:

### 1'3-diethylthia-2'-cyanine chloride

### 1,1'-diethyl-2,2'-cyanine chloride

### 3,3'-diethyloxacarbocyanine iodide

### 5,5'-dichloro-3,3'-diethylthiacarbocyanine iodide

### 1,1'-diethyl-2,2'-carbocyanine iodide

### 3,3'-diethylthiazolocarbocyanine iodide

### 3,3'-diethyl-4,4'-diphenylthiazolocarbocyanine iodide

3,3'-diethyl-9-methylthiacarbocyanine iodide  
 1,3,3'-triethylbenzimidazolo-oxacarbocyanine iodide  
 5-chloro-1,3,3'-triethylbenzimidazolo-oxacarbocyanine iodide  
 5,6-dichloro-1,3,3'-triethylbenzimidazolothiacarbocyanine iodide  
 1,1',3-triethylbenzimidazolo-2'-carbocyanine iodide  
 1,1',3-triethylbenzimidazolo-40'-carbocyanine iodide  
 1,1'-diethyl-2,4'-carbocyanine iodide  
 1',3-diethyl-4-methylthiazolo-2'-carbocyanine iodide  
 3,3'-diethylthiadicarbocyanine iodide  
 1,1'-diethyl-2,2'-dicarbocyanine iodide  
 1',3-diethylthia-2'-dicarbocyanine iodide  
 Anhydro-5,5',6,6-tetrachloro-1,1',3-triethyl-3'-(4-sulfobutyl)benzimidazolocarbocyanine hydroxide  
 Anhydro-5,6-dichloro-b1-ethyl-3-(3-sulfobutyl)-3'-(3-sulfopropyl)-4',5'-benzobenzimidazolothiacarbocyanine hydroxide  
 1,1',3,3'-tetraethyl-naphtho[1,2-d]imidazolocarbocyanine iodide  
 Anhydro-5,6-dichloro-1,3-diethyl-(3'-sulfobutyl)benzimidazoloselenacarbocyanine hydroxide  
 1,2-diethylthia-4'-carbocyanine iodide  
 Anhydro-5,5',6,6'-tetrachloro-1,1'-diethyl-3,3'-di(4-sulfobutyl)benzimidazolocarbocyanine hydroxide

Especially useful cyanine dyes include the carbocyanine, dicarbocyanine and tricarbocyanine dyes. Cyanine dyes which have at least one nucleus selected from a 5- or 6-dichlorobenzimidazole nucleus, a 5- or 6-methoxy-substituted benzothiazole nucleus or a 5- or 6-trifluoromethylbenzimidazole nucleus provide particularly good results. Supersensitization of these dyes with a sulfonated polynuclear aromatic organic supersensitizer, an azaindene or a silver halide reducing agent (e.g., those described below) is sometimes advantageous.

40 A particularly useful class of cyanine dyes are tricarbocyanine dyes in which the meso carbon atom of the methine linkage of the dye is attached to the nitrogen atom of an amino group which forms an enamine with the methine linkage of the tricarbocyanine dye. The term "tricarbocyanine" denotes dyes having the amidinium-ion chromophoric system (see Mees and James, *The Theory of the Photographic Process*, Third Edition, 1966, page 201). Typically, such dyes have 45 two nitrogen-containing heterocyclic nuclei which are joined by a straight chain methine linkage having seven methine groups. The carbon atom of the central methine group of the methine linkage is referred to herein 50 as the meso carbon atom of the methine linkage.

The word "enamine" is used herein to refer to the group



See *Advances in Organic Chemistry, Methods and Results*, Volume 4, Raphael, Taylor and Wynberg, 1963, Interscience, page 3, and Fieser and Fieser, <sup>60</sup> *Advanced Organic Chemistry*, Reinhold Publishing Corp., 1961, pages 494-499.

The preferred enamine tricarbocyanine dyes used herein have the following formula:



wherein  $a$  and  $b$  each represents an integer of from 1 to 2;  $X_1$  represents an acid anion, such as those mentioned above;  $R_3$  and  $R_4$  each represents a value given for  $R_1$  and  $R_2$  above;  $Z_2$  and  $Z_3$  are each selected from a value given for  $Z$  and  $Z_1$  above;  $Q^1$  represents a divalent linkage, such as ethylene, trimethyl, orthophenylene, which linkage can be substituted, for example, with halogen, an alkyl or an alkoxy group of one to four carbon atoms; and  $R_5$  and  $R_6$  taken separately each represents a member selected from the group consisting of alkyl and aryl, and, taken together  $R_5$  and  $R_6$  represent the non-metallic atoms required to complete a heterocyclic ring containing from 5 to 6 atoms, e.g., a morpholino group, a thiomorpholino group, a piperidino group, a piperazinyl group, (preferably a 4-alkyl-1-piperazinyl group such as methyl, ethyl, ethoxycarbonyl, propyl or butyl groups, or an 4-aryl-1-piperazinyl group such as a 4-phenyl-1-piperazinyl group) a pyrrolidinyl group, an indolyl group, a tetrahydroquinolyl group and a decahydroquinolyl group. Especially good results are obtained when  $Z_2$  and  $Z_3$  each represents a benzoxazole, a naphthothiazole nucleus, or a benzothiazole nucleus;  $Q^1$  represents an ethylene linkage; and,  $R_5$  and  $R_6$  are taken together and represents a piperazinyl group, 4-ethoxycarbonyl-1-piperazinyl being preferred.

Typical specific enamine tricarbocyanine dyes useful in the practice of this invention are set out in Table A below:

TABLE A

|      |                                                                                                                                                                                                               |
|------|---------------------------------------------------------------------------------------------------------------------------------------------------------------------------------------------------------------|
| I    | 11-(4-Ethoxycarbonyl-1-piperazinyl)-3,3'-diethyl-10,12-ethyleneoxatricarbocyanine perchlorate                                                                                                                 |
| II   | 3,3'-Diethyl-10,12-ethylene-11-(4-methyl-1-piperazinyl)oxatricarbocyanine perchlorate                                                                                                                         |
| III  | 3,3'-Diethyl-10,12-ethylene-11-(4-methyl-1-piperazinyl)thiaticarbocyanine perchlorate                                                                                                                         |
| IV   | 11-(4-Ethoxycarbonyl-1-piperazinyl)-3,3'-diethyl-10,12-ethylene-5,5'-diphenyloxatricarbocyanine perchlorate                                                                                                   |
| V    | Anhydro-11-(4-ethoxycarbonyl-1-piperazinyl)-10,12-ethylene-3,3'-di(3-sulfopropyl)thiaticarbocyanine hydroxide                                                                                                 |
| VI   | Anhydro-10,12-ethylene-11-(4-methyl-piperazinyl)-3,3'-di(3-sulfopropyl)oxatricarbocyanine hydroxide                                                                                                           |
| VII  | Anhydro-10,12-ethylene-11-(4-methyl-1-piperazinyl)-3,3'-di(3-sulfopropyl)thiaticarbocyanine hydroxide                                                                                                         |
| VIII | 11-(4-Ethoxycarbonyl-1-piperazinyl)-3,3'-diethyl-10,12-ethylenethiaticarbocyanine perchlorate                                                                                                                 |
| IX   | 11-(4-phenyl-1-piperazinyl)-3,3'-diethyl-10,12-orthophenylenethiaticarbocyanine p-toluene sulfonate<br>Anhydro-11-dibutylamino-10,12-ethylene-3,3'-di(3-sulfopropyl)thiaticarbocyanine hydroxide, sodium salt |
| XI   | 3,3'-Diethyl-10,12-ethylene-11-(1-pyrrolidinyl)thiaticarbocyanine iodide                                                                                                                                      |
| XII  | 10,12-ethylene-1,1',3,3,3',3'-hexamethyl-11-(1-pyrrolidinyl)indotricarbocyanine iodide                                                                                                                        |
| XIII | 3,3'-Diethyl-10,12-ethylene-11-piperidion-thiaticarbocyanine iodide                                                                                                                                           |
| XIV  | 3,3'-Diethyl-10,12-ethylene-1-morpholinothiaticarbocyanine iodide                                                                                                                                             |
| XV   | 3,3'-Diethyl-11-piperidino-10,12-trimethylenethiaticarbocyanine iodide                                                                                                                                        |
| XVI  | 3,3'-Diethyl-10,12-ethylene-11-(1-idolyl)oxatricarbocyanine perchlorate                                                                                                                                       |

|  |       |                                                                                                                                                       |   |
|--|-------|-------------------------------------------------------------------------------------------------------------------------------------------------------|---|
|  |       |                                                                                                                                                       | 8 |
|  |       | 3,3'-Diethyl-10,12-ethylene-11-[1-(1,2,3,4-tetrahydroquinolyl)oxyatricarbocyanine perchlorate                                                         |   |
|  | XVII  | 11-Diethylamino-3,3'-diethyl-10,12-ethylene-thiaticarbocyanine perchlorate                                                                            |   |
|  | XVIII | 11-Diethylamino-10,12-ethylene-1,11,3,3'-hexamethylindotricarbocyanine perchlorate                                                                    |   |
|  | XIX   | 3,3'-Diethyl-10,12-ethylene-11-[1-(1,2,3,4-tetrahydroquinolyl)4,5,4',5'-dibenzothiaticarbocyanine perchlorate                                         |   |
|  | XX    | 11-Diphenylamino-3,3'-diethyl-10,12-ethyleneoxatricarbocyanine perchlorate                                                                            |   |
|  | XXI   | 11-Dimethylamino-3,3'-diethyl-10,12-ethylenethiaticarbocyanine perchlorate                                                                            |   |
|  | XXII  | 3,3'-Diethyl-10,12-trimethylene-11-thiomorpholinoxathiacarbocyanine perchlorate                                                                       |   |
|  | XXIII | 3,3'-Diethyl-10,12-ethylene-11-(1-decahydroquinolyl)-4,4'-tricarbocyanine perchlorate                                                                 |   |
|  | XXIV  | Anhydro-11-(4-ethoxycarbonyl)piperazin-1-yl)-10,12-ethylene-3,3'-bis(3-sulfopropyl)-5,6,5',6'-dibenzothiaticarbocyanine hydroxide, triethylamine salt |   |
|  | XXV   |                                                                                                                                                       |   |

20 The enamine tricarbocyanine dyes employed in this invention can be prepared by reacting one mol of an intermediate having formula III below:



30 with one mol of an enamine salt of formula IV below:



to obtain a compound having formula V below:



45 One mol of the compound of formula V above can then be reacted with one mol of a compound having formula VI below:



55 to obtain a compound having formula II above. In the above formulas,  $X_1$ ,  $a$ ,  $b$ ,  $Z_2$ ,  $Z_3$ ,  $Q^1$ ,  $R_3R_4$ ,  $R_5$  and  $R_6$  have the meanings given above. The reactions are advantageously conducted in a suitable solvent, such as acetone or acetic anhydride, and preferably in the presence of a basic condensing agent, such as triethylamine, and at elevated temperatures, such as the refluxing temperature of the reaction mixtures. Further details on the preparation of dyes employed in this invention appear in Jeffreys U.S. Pat. application Ser.

60 No. 314,864 filed Oct. 10, 1963 U.S. Pat. No. 3483195 and corresponding French Pat. No. 1,410,864; Jeffreys

U.S. Pat. application Ser. No. 518,010 filed Jan. 3, 1966 U.S. Pat. No. 3506655, and corresponding Belgian Pat. No. 674,800; Fumia et al. U.S. Pat. application Ser. No. 574,947 filed Aug. 25, 1966 Pat. No. 3482978 and corresponding Belgian Pat. No. 702,840; and, Fumia et al. U.S. Pat. application Ser. No. 860,395 filed Sept. 23, 1969 now abandoned, and entitled "Sensitizing Dyes and Photographic Emulsions and Elements Containing Said Dyes," and continuation-in-part application thereof U.S. Pat. Ser. No. 22,708 filed Mar. 25, 1970 Pat. No. 3623881. Supersensitization of these dyes with a sulfonated polynuclear aromatic organic supersensitizer, an azaindene or a silver halide reducing agent is described by Hiller et al in U.S. Pat. application Ser. No. 860,394 filed Sept. 23, 1969 now abandoned.

Merocyanine dyes are effectively employed in the practice of this invention. Typical useful merocyanine dyes have the following formula:



wherein  $\text{R}_7$ ,  $\text{L}$  and  $\text{Z}_4$  represents a value selected from those given above for  $\text{R}_1$ ,  $\text{L}$  and  $\text{Z}$ , respectively;  $c$  represents an integer of from 1 to 2;  $p$  represents an integer of from 1 to 3; and,  $\text{Q}$  represents the non-metallic atoms necessary to complete a 5- or 6-membered nucleus of the type used in merocyanine dyes typically containing a hetero atom selected from nitrogen, sulfur, selenium, and oxygen, such as a 2-pyrazolin-5-one nucleus, e.g., 3-methyl-1-phenyl-2-pyrazolin-5-one, 1-phenyl-2-pyrazoline-5-one, 1-(2-benzothiazolyl)-3-methyl-2-pyrazolin-5-one, etc.; an isoxazolone nucleus, e.g., 3-phenyl-5(4H)-isoxazolone, 3-methyl-5(4H)-isoxazolone, etc.; an oxindole nucleus, e.g., 1-alkyl-2-oxindoles, etc.; a 2,4,6-triketohexahydroprymidine nucleus, e.g., barbituric acid or 2-triobarbituric acid as well as their 1-alkyl (e.g., 1-methyl, 1-ethyl, 1-propyl, 1-heptyl, etc.) or 1,3-dialkyl (e.g., 1,3-dimethyl, 1,3-diethyl, 1,3-dipropyl, 1,3-diisopropyl, 1,3-dicyclohexyl, 1,3-di( $\beta$ -methoxyethyl), etc.; or 1,3-diaryl (e.g., 1,3-diphenyl, 1,3-di-(p-chlorophenyl), 1,3-di(p-ethoxycarbonylphenyl), etc.); or 1-aryl (e.g., 1-phenyl, 1-p-chlorophenyl, 1-p-ethoxycarbonylphenyl), etc.) or 1-alkyl-3-aryl (e.g., 1-ethyl-3-phenyl, 1-n-heptyl-3-phenyl, etc.) derivatives; a rhodanine nucleus (i.e., 2-thio-2,4-thiazolidinedione series), such as rhodanine, 3-alkylrhodanines, e.g., 3-ethylrhodanine, 3-allylrhodanine etc., 3-carboxyalkylrhodanines, e.g., 3-(2-carboxyethyl)rhodanine, 3-(4-carboxybutyl)rhodanine, etc., 3-sulfoalkylrhodanines, e.g., 3-(2-sulfoethyl)rhodanine, 3-(3-sulfopropyl)rhodanine, 3-(4-sulfobutyl)rhodanine, etc., or 3-arylrhodanines, e.g., 3-phenylrhodanine, etc., etc.; a 2(3H)-imidazo[1,2-a]pyridone nucleus; a 5,7-dioxo-6,7-dihydro-5-thiazolo[3,2-a]pyrimidine nucleus, e.g.,

5,7-dioxo-3-phenyl-6,7-dihydro-5-thiazolo[3,2-a]-pyrimidine, etc.; a 2-thio-2,4-oxazolidinedione nucleus (i.e., those of the 2-thio-2,4(3H, 5H)-oxazoleidine series) e.g., 3-ethyl-2-thio-2,4-oxazolidinedione, 3-(2-sulfoethyl)-2-thio-2,4-oxazolidinedione, 3-(4-sulfobutyl)-2-thio-2,4-oxazolidinedione, 3-(3-carboxypropyl)-2-thio-2,4-oxazolidinedione, etc.; a thianaphthenone nucleus, e.g., 3-(2H)-thianaphthenone, etc.; a 2-thio-2,5-thiazolidinedione nucleus (i.e., the 2-thio-2,5-(3H,4H)-thiazoleidine se-

ries), e.g., 3-ethyl-2-thio-2,5-thiazolidinedione, etc; a 2,4thiazolidinedione nucleus, e.g., 2,4-thiazolidinedione, 3-ethyl-2,4thiazolidinedione, 3-phenyl-2,4-thiazolidinedione, etc; a thiazolidinone nucleus, e.g., 4-thiazolidinone, 3-ethyl-4-thiazolidinone, 3-phenyl-4-thiazolidinone, 3- $\alpha$ -naphthyl-4-thiazolidinone, etc; a 2-thiazolin-4-one nucleus, e.g., 2-ethylmercapto-2-thiazolin-4-one, 2-alkylphenylamino-2-thiazolin-4-one, 10 2-diphenylamino-2-thiazolin-4-one, etc; a 2-imino-4-oxazolidinone (i.e., pseudohydantoin) nucleus; a 2,4-imidazolidinedione (hydantoin) nucleus, e.g., 2,4-imidazolidinedione, 3-ethyl-2,4-imidazolidinedione, 3-phenyl-2,4-imidazolidinedione, 3- $\alpha$ -naphthyl-2,4-imidazolidinedione, 1,3-diethyl-2,4-imidazolidinedione, 1-ethyl-3-phenyl-2,4-imidazolidinedione, 1-ethyl-3- $\alpha$ -naphthyl-2,4-imidazolidinedione, 1,3-diphenyl-2,4-imidazolidinedione, etc; a 2-thio-2,4-imidazolidinedione (i.e., 2-thiohydantoin) nucleus, e.g., 2-thio-2,4-imidazolidinedione, 3-ethyl-2-thio-2,4-imidazolidinedione, 3-(4-sulfobutyl)-2-thio-2,4-imidazolidinedione, 3-(2-carboxyethyl)-2-thio-2,4-imidazolidinedione, 3-phenyl-2-thio-2,4-imidazolidinedione, 3- $\alpha$ -naphthyl-2-thio-2,4-imidazolidinedione, 1,3-diethyl-2-thio-2,4-imidazolidinedione, 1-ethyl-3-phenyl-2-thio-2,4-imidazolidinedione, 1-ethyl-3- $\alpha$ -naphthyl-2-thio-2,4-imidazolidinedione, 1,3-diphenyl-2-thio-2,4-imidazolidinedione, etc.; a 2-imidazolin-5-one nucleus, e.g., 2-propylmercapto-2-imidazolin-5-one, etc.; etc. (Especially useful are nuclei wherein  $\text{Q}$  represents the non-metallic atoms required to complete a heterocyclic nucleus containing five to six atoms in the heterocyclic ring, three to four of said atoms being carbon, and two of said atoms being selected from the group consisting of nitrogen, oxygen, and sulfur, and at least one of said two atoms being a nitrogen atom. Typical useful merocyanine dyes are described in Brooker et al. U.S. Pat. No. 2,493,747 and 2,493,748, both issued Jan. 10, 1950, and Knott U.S. Pat. No. 2,839,403 issued June 17, 1958.

Another preferred class of methine dyes include those comprising first and second nuclei joined by a double bond or methine linkage (including one or more methine groups); the first of said nuclei being selected from the group consisting of (1) a nitrogen-containing heterocyclic nucleus of the type used in cyanine dyes having from 5 to 6 non-metallic atoms in the heterocyclic ring, and (2) a nitrogen-containing heterocyclic ketomethylene nucleus of the type used in merocyanine dyes having from 5 to 6 non-metallic atoms in the heterocyclic ring, joined in each instance by a carbon atom of (1) or (2) to said linkage; and said second nucleus being an enamine group selected from the group consisting of a 1-(3,4,4a,5,6,7-hexahydro-2-naphthyl)-pyrrolidine group, a 1-(3,3a,4,5-tetrahydro-2H-inden-6-yl)pyrrolidine group, a 1-(2-norbornylidene)pyrrolidine group and a 1-(1-indanylidene)pyrrolidine group, joined at a carbon atom thereof to said linkage, to complete said dye. Preferred dyes of this type include those represented by the following formulas:



and

IX.



wherein  $e$  and  $g$  represents a positive integer of from 1 to 2;  $f$  represents a positive integer of from 1 to 3;  $L$  represents a methine linkage, e.g.,  $=\text{CH}-$ ,  $=\text{C}(\text{CH}_3)$ ,  $=\text{C}(\text{C}_6\text{H}_5)$ , etc.;  $D$  represents an enamine group selected from a 2,3,4,4a,5,6-hexahydro-7-(1-pyrrolidinyl)-1-naphthyl group, a 2,6,7,7a-tetrahydro-5-(1-pyrrolidinyl)-3-indenyl group, a 3-(1-pyrrolidinyl)-2-norbornen-2-yl group or a 3-(1-pyrrolidinyl)-2-indenyl group, represented by the following basic structures:



and



which groups can be further substituted on appropriate nuclear carbon atoms thereof by alkyl, e.g., methyl, butyl, etc., or alkoxy, e.g., methoxy, butoxy, etc., and the like;  $R_8$ ,  $X_2$  and  $Q_1$  represents a value given above for  $R_1$ ,  $X$  and  $Q$ , respectively. Methine dyes of this type can be conveniently prepared in a number of ways. For example, a number of the dyes defined by formula VIII above are advantageously prepared by heating a mixture of (1) a heterocyclic salt of the formula:

X.



wherein  $f$  is 2 or 3;  $e$ ,  $L$ ,  $R_8$ ,  $X_2$  and  $Z_5$  are as previously defined, and  $R_9$  represents a hydrogen atom or an acyl group, e.g., acetoxy, phenoxy, etc., with (2) an enamine intermediate selected from the group consisting of a 1(3,4,4a,5,6,7-hexahydro-2-naphthyl)pyrrolidine,

or a 1-(3,3a,4,5-tetrahydro-2H-inden-6-yl)pyrrolidone, or a 1-(2-norbornylidene)pyrrolidinium salt, e.g., the chloride, bromide, iodide, perchlorate, p-toluenesulfonate, etc. salt, or a 1-(1-indanylidene)pyrrolidinium salt, e.g., the chloride, bromide, iodide, perchlorate, p-toluenesulfonate, etc. salt, in approximately equimolar proportions, in a solvent medium such as ethanol, pyridine, N,N-dimethylacetamide, acetic anhydride, etc. etc. Advantageously, a basic condensing agent such as triethylamine is used with the acetic anhydride reaction medium. The dyes are then separated from the reaction mixtures and purified by one or more recrystallizations from appropriate solvents such as methanol, mixtures of pyridine and methanol, and the like. The dyes wherein the value of  $f$  is 1 in formula VIII above are advantageously prepared with (1) a heterocyclic salt of the formula:

20 XI.



wherein  $g$ ,  $R_8$ ,  $X_2$  and  $Z_5$  are as previously defined and  $R_{10}$  represents an alkyl or aryl group, e.g., methyl, butyl, phenyl, etc., and (2) an enamine intermediate above defined, under generally similar reaction conditions and purification of the dyes as described in the preceding procedure. The dyes defined by formula IV above are also prepared by the above procedure described for the dyes of formula VIII using the same enamine intermediates except that the heterocyclic salt of formula X is replaced by a ketomethylene heterocyclic compound of the formula:

35

XII.



40

wherein  $g$ ,  $L$ ,  $R_9$  and  $Q_1$  are as previously defined. Dyes of this type are described in Fumia et al. U.S. Pat. application Ser. No. 830,483 filed June 4, 1969, and include such dyes as 3-ethyl-2-

45 {2-[2,3,4,4a,5,6-hexahydro-7-(1-pyrrolidinyl)-1-naphthyl]vinyl} benzoxazolium iodide; 3-ethyl-2-[2-[2,3,4,4a,5,6-hexahydro-7-(1-pyrrolidinyl)-1-naphthyl]methylene] benzothiazolium iodide; 3-ethyl-5-[2,3,4,4a,5,6-hexahydro-7-(1-pyrrolidinyl)-1-naphthyl]methylene} rhodanine; 3-ethyl-2-[2,6,7,7a-tetrahydro-5-(1-pyrrolidinyl)-3-indenyl]benzothiazolium perchlorate; 3-ethyl-2-[2,6,7,7a-tetrahydro-5-(1-pyrrolidinyl)-3-indenyl]-vinyl} benzoxazolium iodide; 3-ethyl-2-[2,6,7,7a-tetrahydro-5-(1-pyrrolidinyl)-3-indenyl]-methylene} benzothiazolium iodide; 3-phenyl-4-[2,6,7,7a-tetrahydro-5-(1-pyrrolidinyl)-3-indenyl]-methylene} 2-isoxazolin-5-one; 3-methyl-1-phenyl-4-[2,6,7,7a-tetrahydro-5-(1-pyrrolidinyl)-3-indenyl]-methylene} 2-pyrazolin-5-one; 3-ethyl-5-[2,56,7,7a-tetrahydro-5-(1-pyrrolidinyl)-3-indenyl]-methylene} rhodanine; 3-ethyl-2-[2-[3-(1-pyrrolidinyl)-2-norbornen-2-yl]vinyl]benzoxazolium perchlorate; 3-ethyl-2-[2-[3-(1-pyrrolidinyl)-2-norbornen-2-yl]vinyl]benzothiazolium perchlorate;

55 3-ethyl-2-[2-[3-(1-pyrrolidinyl)-2-norbornen-2-yl]vinyl]benzoxazolium perchlorate; 3-ethyl-2-[2-[3-(1-pyrrolidinyl)-2-norbornen-2-yl]vinyl]benzothiazolium perchlorate; 1-ethyl-2-[2-[3-(1-pyrrolidinyl)-2-norbornen-2-yl]vinyl]

naphtho[1,2-d]thiazolium perchlorate; 1,3,3-trimethyl-2-{2-[3-(1-pyrrolidinyl)-2-indenyl]vinyl}-3H-indolium perchlorate; 3-ethyl-2-{2-[3-(1-pyrrolidinyl)-2-indenyl]vinyl}-benzoxazolium perchlorate; 3-ethyl-2-{2-[3-(1-pyrrolidinyl)-2-indenyl]vinyl}benzothiazolium perchlorate and 1-ethyl-2-{2-[3-(1-pyrrolidinyl)-2-indenyl]vinyl}naphtho[1,2-d]thiazolium perchlorate.

Another highly useful class of dyes are enamine 10  
methine dyes which contain a double bond remote  
from the chromophoric chain. Such useful enamine  
dyes include cyanine, hemicyanine and hemioxonol  
dyes. Such dyes can have formula II above wherein R<sub>5</sub>  
and R<sub>6</sub>, taken separately, each represents an allyl 1  
group, or R<sub>5</sub> and R<sub>6</sub>, taken together, represent the  
atoms required to complete a 1,2,5,6-tetrahydro-1-  
pyridyl nucleus or a 3-pyrrolin-1-yl nucleus. Other dyes  
of this class include those represented by formulas VIII  
and IX above wherein D represents a group having one 2  
of the following formulas:



Still other useful dyes of this class have the following formula:



wherein  $Q_2$  represents a value selected from those given for  $Q_1$  above and  $D_1$  represents a group having the following formula: 5



Enamine dyes containing a double bond remote from the chromophoric chain can be prepared in a manner similar to the preparation of the enamine dyes of formulas II, VIII and IX above, but using one of the following starting materials:

### Intermediate A — 1-cyclopentylidene-3-pyrrolinium perchlorate



10 3-Pyrrolinium perchlorate (17.0 g) and 3-pyrrolidine (4 drops) are suspended in ethanol (75 ml) and the suspension heated on a steam bath to obtain a solution. Cyclopentanone (10.1 g) is then added to the hot solution and solid precipitated. The mixture is heated to reflux and then chilled. The solid is collected on a filter and the yield is 22.5 g (95 percent), m.p. = 202°–203°  
 15 *Caution*

### C.dec.

Intermediate B — 1-Isopropylidene-3-pyrrolinium perchlorate



30 A solution of 3-pyrroline (14.5 g) in ether (1 l.) is treated with 72 percent perchloric acid (28.0 g) with stirring and cooling. Decanted, stirred residue with a fresh portion of ether (1 l.), decanted and then suspended the residue in ethanol (125 ml). Acetone (11.6 g) is added, the mixture is heated to reflux and then chilled. The solid is collected on a filter and then 35 crystallized from ethanol. The yield is 28 g (67 percent), m.p. = 168°-169° C dec. In preparing dyes from this compound, it is necessary to have acetic anhydride present which indicates that the compound may be a hydrate.

#### 40 Intermediate C — Cyclopentenylidenediallylammonium perchlorate



55      Cyclopentanone (25.2 g), diallylamine (49.0 g), p-toluene sulfonic acid (0.5 g) and benzene (90 ml) are placed in an apparatus designed for the continuous removal of water and heated at reflux for 16 hours. After evaporation under reduced pressure, the residue is distilled in vacuum to yield the enamine (b.p. ~93° C/15 mm Hg). The enamine so obtained is dissolved in ether (1 l.), and the cooled solution treated with 72 percent perchloric acid until the mixture is just acid. Decanted, 60 stirred residue with a fresh portion of ether (1 l.), decanted and then recrystallized the solid from ethanol. 65 The yield is 42.8 g (54 percent), m.p. = 122°-123° C dec.

15

Intermediate D — 1-(5,5-Dimethyl-3-methylene-1-cyclohexen-1-yl)-3-pyrroline



Isophorone (41.4 g), 3-pyrroline (31.0 g), p-toluene sulfonic acid (0.5 g) and benzene (90 ml) are placed in an apparatus designed for the continuous removal of water and heated at reflux for 1 hour. After evaporating under reduced pressure, the residue is distilled in vacuum. Decomposition takes place during the distillation with 12.1 g (21 percent) of the desired material being obtained. (b.p. = 89°–95° C/0.4–1.1 mm Hg)

Intermediate E — 5,5-Dimethyl-3-(3-pyrrolin-1-yl)-2-cyclohexen-1-one



5,5-Dimethyl-1,3-cyclohexanedione (28.0 g), 3-pyrroline (15.2 g) and benzene (250 ml) are placed in an apparatus designed for the continuous removal of water and heated at reflux for 1 hour. The mixture is then evaporated, under reduced pressure, to a volume of ~100 ml. The residue is diluted to ~400 ml with ligroine (b.p. 35°–60°) and the mixture chilled. The solid is collected on a filter and the yield is 37.5 g (96 percent), m.p. = 111°–112° C. dec.

Intermediate F — 1-(3-Chloro-5,5-dimethyl-2-cyclohexen-1-ylidene)-3-pyrrolinium perchlorate



To a solution of 5,5-dimethyl-3-(3-pyrrolin-1-yl)-2-cyclohexen-1-one (37.5 g) in benzene (300 ml) is added phosphorous pentachloride (40.8 g). The mixture is heated to reflux and then removed from heat until the initial reaction has subsided. The reaction is then heated at reflux for 2 1/4 hours. After cooling, the mixture is stirred with ice water (~300 ml). The water layer is removed and an aqueous solution of sodium perchlorate (36 g/100 ml) is added to it. After chilling, the solid is collected on a filter and dried. The crude yield is 40.5 g (67 percent). After one recrystallization from ethanol, the yield is 29.5 g (49 percent), m.p. = 140°–141° C dec.

Intermediate G — 1-Cyclopentylidene-1,2,5,6-tetrahydropyridinium perchlorate

5



1,2,5,6-Tetrahydropyridine (8.7 g) and cyclopentanone (10.7 g) are dissolved in ethanol (25 ml) and the solution treated with 72 percent perchloric acid (14.0 g) with cooling. The mixture is then heated at reflux for 15 minutes and, after chilling, the solid is collected on a filter. The yield is 16.6 g (66 percent), m.p. = 230°–231° C dec.

Representative useful enamine dyes having a double bond remote from the chromophoric chain, and the preparation thereof, are given below:

3-Ethyl-2-[4-(3-pyrrolin-1-yl)-3,4-trimethylene-1,3-butadienyl]-benzoxazolium perchlorate

25



30

1-Cyclopentylidene-3-pyrrolinium perchlorate (1.3 g), 2-(2-acetanilidovinyl)-3-ethylbenzoxazolium iodide (2.2 g), and triethylamine (1.5 ml) are dissolved in acetic anhydride (15 ml) and stirred at room temperature for 15 minutes. The solid is collected on a filter and, after two recrystallizations from methanol, the yield of purified dye is 0.5 g (25 percent), m.p. = 262°–263° C dec.

3,3'-Diethyl-10,12-ethylene-11-(3-pyrrolin-1-yl)oxatricarbocyanine perchlorate

45



55

1-Cyclopentylidene-3-pyrrolinium perchlorate (1.2 g), 2-(2-acetanilidovinyl)-3-ethylbenzoxazolium iodide (4.8 g), and triethylamine (1.5 ml) are dissolved in acetic anhydride (15 ml) and heated at reflux for 10 minutes. After cooling to room temperature, the solid is collected on a filter, washed with methanol and then recrystallized from cresol/methanol. The yield of purified dye is 0.5 g (22 percent), m.p. = 267°–268° C dec.

3-Ethyl-2-[4-(3-pyrrolin-1-yl)-1,3-pentadienyl]benzoxazolium perchlorate

65

17



1-Isopropylidene-3-pyrrolinium perchlorate (2.3 g), 2-(2-acetanilidovinyl)-3-ethylbenzoxazolium iodide (4.3 g), acetic anhydride (1.0 ml) and triethylamine (1.7 ml) are dissolved in ethanol (20 ml) and heated at reflux for 10 minutes. After chilling, the solid is collected on a filter and then recrystallized from methanol. The yield of purified dye is 1.1 g (29 percent), m.p. = 223°-224° C dec.

3-Methyl-2-[4-(3-pyrrolin-1-yl)-1,3-pentadienyl]thiazolium perchlorate

1-Isopropylidene-3-pyrrolinium perchlorate (2.3 g), 2-(2-anilinovinyl)-3-methyl-2-thiazolium iodide (3.5 g), acetic anhydride (2.0 ml), and triethylamine (3.4 ml) are dissolved in acetonitrile (20 ml) and heated at reflux for 10 minutes. After chilling, the solid is collected on a filter and then recrystallized from methanol. The yield of purified dye is 1.2 g (36 percent), m.p. = 223°-224° C dec.

2-[2-(2-Diallylamino-1-cyclopentenyl)vinyl]-3-ethylbenzothiazolium perchlorate



Cyclopentenylidenediallylammonium perchlorate (2.9 g), 2-(2-acetanilidovinyl)-3-ethylbenzothiazolium iodide (4.5 g) and triethylamine (1.4 ml) are dissolved in acetonitrile (15 ml) and heated at reflux for 5 minutes. After chilling, the crude dye is collected on a filter and recrystallized from methanol with the methanol solution being treated with norite. The yield of purified dye is 1.47 g (33 percent), m.p. = 219°-220° C dec.

11-Diallylaminoo-3,3'-diethyl-10,12-ethylenoatricarbocyanine perchlorate



18

Cyclopentenylidenediallylammonium perchlorate (1.32 g), 2-(2-acetanilidovinyl)-3-ethylbenzoxazolium iodide (4.56 g) and triethylamine (1.5 ml) are dissolved in N,N-dimethylacetamide (10 ml) and heated at a gentle reflux for 5 minutes. The reaction mixture is diluted to ~300 ml with boiling methanol and, after chilling, the dye is collected on a filter (0.97 g, 32 percent). After one recrystallization from methanol, the 10 yield of purified dye is 0.64 g (21 percent), m.p. = 229°-230° C dec.

5-(2-Diallylamino-1-cyclopentenyl)methylene-3-ethylrhodanine

15



25

5-Acetanilidomethylene-3-ethylrhodanine (3.06 g), cyclopentenylidenediallylammonium perchlorate (2.64 g) and triethylamine (1.5 ml) are dissolved in N,N-dimethylacetamide (15 ml) and heated at a gentle reflux for 5 minutes. The reaction mixture is diluted to 300 ml with boiling methanol and, after chilling, the dye is collected on a filter. The yield is 0.40 (12 percent), m.p. = 127°-128° C dec.

3-Ethyl-2-[4,6-neopentylene-6-(3-pyrrolin-1-yl)-1,3,5-hexatrienyl]benzothiazolium iodide

40



1-(5,5-Dimethyl-3-methylene-1-cyclohexen-1-yl)-3-pyrroline (1.0 g) and 2-(2-acetanilidovinyl)-3-ethylbenzothiazolium iodide (2.3 g) are dissolved in ethanol (15 ml) and heated at reflux for 5 minutes. After chilling, the solid is collected on a filter and dried. The crude yield is 1.4 g (56 percent). After one recrystallization from methanol, the yield of purified dye is 1.1 g (44 percent), m.p. = 233°-234° C dec.

1,3,3-Trimethyl-2-[4,6-neopentylene-6-(3-pyrrolin-1-yl)-1,3,5-hexatrienyl]-3H-indolium perchlorate

60

1-(5,5-Dimethyl-3-methylene-1-cyclohexen-1-yl)-3-pyrroline (1.0 g) and 2-(2-acetanilidovinyl)-1,3,3-trimethyl-3H-indolium iodide (2.2 g) are dissolved in ethanol (15 ml) and heated at reflux for 5 minutes. An aqueous solution of sodium perchlorate (1.0 g/5 ml) is added and, after chilling, the crude dye is collected on a filter. After one recrystallization from methanol, the yield of purified dye is 0.5 g (21 percent), m.p. = 231°-232° C dec.

19

3-Ethyl-5-[3,5-neopentylene-5-(3-pyrrolin-1-yl)-2,4-pentadienylidene]rhodanine



5-Acetanilidomethylene-3-ethylrhodanine (3.1 g) and 1-(5,5-dimethyl-3-methylene-1-cyclohexen-1-yl)-3-pyrroline (2.1 g) are dissolved in N,N-dimethylacetamide (15 ml) and heated at a gentle reflux for 5 minutes. After diluting with ~300 ml of boiling methanol, the mixture is allowed to stand at room temperature for 30 minutes and then the dye is collected on a filter. The yield is 1.0 g (28 percent), m.p. = 219°-220° C dec.

3-Ethyl-5-[5,5-dimethyl-3-(3-pyrrolin-1-yl)-2-cyclohexenylidene]-rhodanine

1-(3Chloro-5,5-dimethyl-2-cyclohexen-1-ylidene)-3-pyrrolinium perchlorate (3.10 g), 3-ethylrhodanine (1.61 g) and triethylamine (3.1 ml) are dissolved in ethanol (20 ml) and heated at reflux for 10 minutes. After chilling, the solid is collected on a filter and then recrystallized from pyridine/methanol. The yield of purified dye is 1.78 g (53 percent), m.p. = 192°-193° C dec.

3-Allyl-5-[5,5-dimethyl-3-(3-pyrrolin-1-yl)-2-cyclohexenylidene]rhodanine



3-Allylrhodanine (1.73 g), 1-(3-chloro-5,5-dimethyl-2-cyclohexen-1-ylidene)-3-pyrrolinium perchlorate (3.10 g) and triethylamine (3.1 ml) are dissolved in ethanol (20 ml) and heated at reflux for 1 minute. The mixture is allowed to stand at room temperature for 30 minutes and then the crude dye is collected on a filter. After one recrystallization from pyridine/methanol, the yield of purified dye is 2.36 g (68 percent), m.p. = 202°-203° C dec.

5-[5,5-Dimethyl-3-(3-pyrrolin-1-yl)-2-cyclohexenylidene]-3-ethyl-1-phenyl-2-thiohydantoin



1-(3-Chloro-5,5-dimethyl-2-cyclohexen-1-ylidene)-3-pyrrolinium perchlorate (3.10 g), 3-ethyl-1-phenyl-2-thiohydantoin (2.2 g) are triethylamine (3.1 ml) are

20

dissolved in ethanol (15 ml) and heated at reflux for 10 minutes. After chilling, the crude dye is collected on a filter and then recrystallized from methanol. The yield of purified dye is 1.50 g (38 percent), m.p. = 219°-220° C dec.

3-Ethyl-2-[4-(1,2,5,6-tetrahydro-1-pyridyl)-3,4-trimethylene-1,3-butadienyl]benzoxazolium perchlorate



10

15

20

1-Cyclopentylidene-1,2,5,6-tetrahydropyridinium perchlorate (2.7 g), 2-(2-acetanilidovinyl)-3-ethylbenzoxazolium iodide (4.3 g) and triethylamine (1.5 ml) are dissolved in acetic anhydride (20 ml) and stirred at room temperature for 2 hours. The crude dye is collected on a filter and then recrystallized from methanol. The yield of purified dye is 0.9 g (21 percent), m.p. = 214°-215° C dec.

3-Ethyl-2-[4-(1,2,5,6-tetrahydro-1-pyridyl)-3,4-trimethylene-1,3-butadienyl]benzothiazolium perchlorate

1-Cyclopentylidene-1,2,5,6-tetrahydropyridinium perchlorate (2.7 g), 2-(2-acetanilidovinyl)-3-ethylbenzothiazolium iodide (4.5 g) and triethylamine (1.5 ml) are dissolved in acetic anhydride (20 ml) and the mixture stirred at room temperature for 1 1/4 hours. The crude dye is collected on a filter, rinsed with ethanol and then recrystallized twice from methanol. The yield of purified dye is 1.0 g (23 percent), m.p. = 227°-228° C dec.

3,3'-Diethyl-10,12-ethylene-11-(1,2,5,6-tetrahydro-1-pyridyl)-oxaticarboxyanine perchlorate

45

50

55

1-Cyclopentylidene-1,2,5,6-tetrahydropyridinium perchlorate (1.2 g), 2-(2-acetanilidovinyl)-3-ethylbenzoxazolium iodide (4.8 g) and triethylamine (1.5 ml) are dissolved in acetic anhydride (20 ml) and heated at reflux for 5 minutes. The hot mixture is turned into a beaker, stirred for 2 minutes and the solid then collected on a filter. After one recrystallization from N,N-dimethylacetamide, the yield of purified dye is 1.1 g (37 percent), m.p. = 251°-252° C dec.

3-Ethyl-5-[2-(3-pyrrolin-1-yl)-1-cyclopentenylmethylen]-rhodanine

1-Cyclopentylidene-1,2,5,6-tetrahydropyridinium perchlorate (1.2 g), 2-(2-acetanilidovinyl)-3-ethylbenzoxazolium iodide (4.8 g) and triethylamine (1.5 ml) are dissolved in acetic anhydride (20 ml) and heated at reflux for 5 minutes. The hot mixture is turned into a beaker, stirred for 2 minutes and the solid then collected on a filter. After one recrystallization from N,N-dimethylacetamide, the yield of purified dye is 1.1 g (37 percent), m.p. = 251°-252° C dec.

3-Ethyl-5-[2-(3-pyrrolin-1-yl)-1-cyclopentenylmethylen]-rhodanine



Cyclopentylidene-3-pyrrolinium perchlorate (2.36 g), 5-acetanilidovinyl-3-ethylrhodanine (3.06 g), and triethylamine (1.5 ml) are dissolved in ethanol (15 ml) and heated at reflux for 5 minutes. After chilling, the crude dye is collected on a filter and, after one recrystallization from benzene, the yield of purified dye is 1.35 g (44 percent), m.p. = 199°–200° C dec.

3-Carboxymethyl-5-[2-(3pyrrolin-1-yl)-1-cyclopentenylmethylene]-rhodanine, sodium salt

1-(2-Anilinomethylenecyclopentylidene)-3-pyrrolinium perchlorate (3.39 g), 3-carboxymethylrhodanine (1.91 g), acetic anhydride (1.0 ml), and triethylamine (3.0 ml) are dissolved in 4-butyrolactone (15 ml) and heated at a gentle reflux for 5 minutes. A solution of sodium iodide (2.00 g) in acetonitrile (50 ml) is added and, after cooling, the crude dye is collected on a filter. After one recrystallization from N,N-dimethylacetamide/acetonitrile and another from water/acetonitrile, the yield is 0.31 g (9 percent), m.p. = 257°–258° C dec.

It is sometimes desirable to supersensitize the dyes employed in this invention. Preferred supersensitizers are the polynuclear aromatic compounds containing at least one sulfo group. The term "polynuclear aromatic" as used herein is intended to mean 2 or more benzene rings fused together (for example, as in naphthalene, pyrene, etc) or at least 2 benzene rings or aromatic rings directly joined together (for example, as in diphenyl, terphenyl, quaterphenyl, etc) or through an aliphatic linkage. Such sulfonated derivatives can conveniently be presented by the following general formula: XIV. T-SO<sub>3</sub>M

wherein T represents a polynuclear aromatic group as defined above and M represents a hydrogen atom or a water-soluble cation salt group (e.g., sodium, potassium, ammonium, triethylammonium, triethanolammonium, pyridinium, etc). Among the most useful of the sulfonated derivatives embraced by Formula XIV above are the compounds represented by the following general formula:

XV.



wherein T<sub>1</sub> represents a 1,3,5-triazin-6-ylamino group, T<sub>2</sub> represents an aromatic group (i.e., benzene or substituted benzene) and M has the values given above.

Typical of the sulfonated derivatives of Formula XV above, wherein T<sub>1</sub> represents a 1,3,5-triazin-2-ylamino group (i.e., a 1,3,5-triazin-2-ylamino group) are the compounds selected from those represented by the following general formula:

XVI.



wherein M has the values given above and R<sub>20</sub>, R<sub>21</sub>, R<sub>22</sub>, R<sub>23</sub> each represents a hydrogen atom or a substituent group, such as hydroxyl, aryloxy (e.g., phenoxy, o-toloxyl, p-sulfophenoxy, etc.), alkoxy (e.g., methoxyl, ethoxyl, etc.), a halogen atom (e.g., chlorine, bromine, etc.), a heterocyclic radical (e.g., morpholinyl, piperidyl, etc.), an alkylthio group (e.g., methylthio, ethylthio, etc.), an arylthio group (e.g., phenylthio, tolylthio, etc.), a heterocyclithio group (e.g., benzothiazylthio, etc.) an amino group, an alkylamino group (e.g., methylamino, ethylamino, propylamino, dimethylamino, diethylamino, dodecylamino, cyclohexylamino, β-hydroxyethylamino, di-β-hydroxyethylamino, β-sulfoethylamino, etc.), an arylamino group (e.g., anilino, o-, m- and p-anisylamino, o-, m- and p-chloroanilino, o-, m- and p-toluidino, o-, m-, and p-carboxyanilino, hydroxyanilino, sulfonaphthylamino, o-, m- and p-aminoanilino, p-acetamidylanilino, etc.), etc.

Compounds of Formula XVI wherein R<sub>20</sub>, R<sub>21</sub>, R<sub>22</sub> and/or R<sub>23</sub> each represents a heterocyclamino group (e.g., 2-benzothiazoleamino, 2-pyridylamino, etc.) can also be used in practicing my invention.

Another group of sulfonated derivatives which are useful in practicing the invention are those represented by the following general formula:

35 XVII.



wherein R<sub>24</sub> is an acylamido group (e.g., acetamido, sulfobenzimidyl, 4-methoxy-3-sulfobenzamido, 2-ethoxybenzamido, 2,4-diethoxy, benzamido, p-tolylamido, 4-methyl-2-methoxybenzamido, 1-naphthoylamino, 2-naphthoylamino, 2,4-dimethoxybenzamido, 2-phenylbenzamido, 2-thienylbenzamido) or a sulfo group, R<sub>26</sub> represents an acylamido group (e.g., as defined by R<sub>24</sub> above), or a sulfoaryl group (e.g., sulfophenyl, p'-sulfodiphenyl, etc.) and R<sub>25</sub> represents a hydrogen atom or a sulfo group, said compound containing at least one sulfo group.

Compounds of Formula XVI which can advantageously be employed in practicing my invention have been described in one or more of the following representative patents: U.S.:

|    |                                                               |                                                                                   |
|----|---------------------------------------------------------------|-----------------------------------------------------------------------------------|
| 60 | 2,171,427<br>2,472,475<br>2,595,030<br>2,660,578<br>2,945,762 | Aug. 29, 1939<br>June 14, 1949<br>Apr. 29, 1952<br>Nov. 24, 1953<br>July 19, 1960 |
|----|---------------------------------------------------------------|-----------------------------------------------------------------------------------|

British:

|    |                                                                |                                                                                                 |
|----|----------------------------------------------------------------|-------------------------------------------------------------------------------------------------|
| 65 | 595,065<br>623,849<br>624,051<br>624,052<br>678,291<br>681,642 | Nov. 26, 1947<br>May 24, 1949<br>May 26, 1949<br>May 26, 1949<br>Sept. 3, 1952<br>Oct. 29, 1952 |
|----|----------------------------------------------------------------|-------------------------------------------------------------------------------------------------|

The products of Formula XVI have been previously employed in the textile field, and are sold under such tradenames as Leucophor B, Calcofluor White MR, Tinopal (SP, WR, BV277, 2B, GS, NG), Blancofor SC, Hiltamine (BSP, N, Sol., 6T6), and the like. 5

The dibenzothiophenedioxide compounds of Formula XVII have, in general, been previously described in the prior art. See, for example, U.S. Pat. Nos. 2,573,652; 2,580,234; and 2,563,493. Further examples of the preparation of such compounds are given in J. E. Jones, J. Spence, and J.A. VanAllan, U.S. Pat. No. 2,937,089, issued May 17, 1960. Still other examples of compounds represented by Formula XIV above which can be used in my invention have been previously described in B. H. Carroll, J. E. Jones, and J. Spence, U.S. Pat. No. 2,950,196, issued Aug. 23, 1960. (See, in particular, the compounds of Formulas II, III and IV of that patent). 15

Compounds selected from those of Formula XV above wherein  $T_1$  represents a 2-benzotriazolyl group can be prepared according to methods previously described in the prior art. See, for example, U.S. Pat. to Zweidler et al. No. 2,713,057, dated July 12, 1955; 25 Keller et al., U.S. Pat. No. 2,684,966, dated July 27, 1954; Zweidler et al., U.S. Pat. No. 2,784,197, dated Mar. 5, 1957; and Keller et al., U.S. Pat. No. 2,784,183, dated Mar. 5, 1956. A somewhat related group of compounds containing a 2-benzotriazolyl 30 group which can be used in this invention have been previously described in U.S. Pat. No. 2,733,165. Such compounds are embraced by Formula IVa above.

Typical sulfonated derivatives embraced by Formulas XIV, XV and XVII and VIa above are (chemical formulas are given for various types to aid in identification): 35

1. a sulfonated triazolostilbene, e.g., of the type shown in U.S. Pat. No. 2,713,057.

(2)



4,4'-di(4'',6''-dihydroxy-2''-s-triazinylamino)stilbene-2,2'-disulfonic acid

3. 4,4'-bis[4-(3'-sulfoanilino)-6-amino-s-triazin-2-ylamino]-stilbene
4. Tinopal-WR, a sulfonated triazinyl stilbene
5. Tinopal-2B, a sulfonated triazinyl stilbene
6. A sulfonated triazinyl stilbene, e.g., of the type shown in U.S. Pat. No. 2,595,030 or British Pat. No. 595,065
7. 4,4'-bis[2-(4-sulfoanilino-2- $\beta$ -hydroxyethylamino)-1,3,5-triazin-6-ylamino]stilbene-2,2'-disulfonic acid
8. 4,4'-bis(2,4-dihydroxy-1,3,5-triazin-6-ylamino)dibenzyl-2,2'-disulfonic acid
9. 4,4'-bis(2- $\beta$ -hydroxyethylamino-4-anilino-1,3,5-triazin-6-ylamino)-1,4-distynylbenzene-2,2'-disulfonic acid
10. 5-methoxy-2-(4-styryl-3-sulfo)phenyl-1,2,3-benzotriazole sodium salt
11. Calcofluor White-MR, a sulfonated triazinyl stilbene



- 10 3,7-bis(2-phenylbenzamido)-2,8-disulfodibenzothiophene-5,5-dioxide
13. 3,7-bis(2-thienylamide)-2,8-disulfodibenzothiophene dioxide sodium salt
14. 3-[4-(4-methoxy-3-sulfobenzamidophenyl)-7-(4-methoxy-3-sulfobenzamido)benzothiophene dioxide sodium salt
15. chrysene-6-sulfonic acid sodium salt
16. pyrene-3-sulfonic acid sodium salt
17. Phenanthrene-3-sulfonic acid sodium salt
18. 2,3-dimethylnaphthalene-1-sulfonic acid sodium salt
19. 4-[4-phenoxy-6-( $\beta$ -hydroxyethylamino)-s-triazin-2-ylamino]4'-[4-chloro-6-di( $\beta$ -hydroxyethylamino)-s-triazin-2-ylamino]-stilbene-2,2'-disulfonic acid
20. 2,8-bis[4-(4-sulfoanilino)-6-hydroxy-s-triazin-2-ylamino]-carbazole
21. 4,4'-bis(4,6-di( $\beta$ -hydroxyethylamino)-s-triazin-2-yl) benzidine-2,2'-disulfonic acid
22. 2-laurylamino-4,6-di(4-sulfoanilino)-s-triazine
23. 4,4'-bis[4-[4'-(N',4''-sulfobenzyl-N'-ethyl)aminoanilino]-6-hydroxy-s-triazin-2-ylamino]stilbene-2,2'-disulfonic acid
24. 5-acetamido-2-(4-styryl-3-sulfo)phenyl-1,2,3-benzotriazole sodium salt
25. 2,7-diacetamido-3,6-disulfodibenzothiophene-5,5-dioxide sodium salt
26. 4-sulfo-o-terphenyl sodium salt (Lour. Organ. Chem., Vol. 14 (1949), pg. 163)
27. pyrene-3-(4-methyl-3-sulfoxytryl)ketone sodium salt
28. 3,7-bis(4-methyl-2-methoxybenzamido)-2,8-disulfodibenzothiophene-5,5-dioxide sodium salt
- 45 As can be seen above, many of the sulfonated derivatives are employed in the form of their water-soluble salts, such as alkali metal (e.g., sodium, potassium, etc.) salts, or ammonium or amine (e.g., triethylamine, triethanolamine, pyridine, aniline, etc.) salts. By thus using these derivatives, they can be added to the emulsions in substantially neutral aqueous solutions without disturbing the pH of the emulsions.
- 50 In accordance with the practice of this invention, any reducing agent (i.e., a material capable of reducing silver halide) can be employed which supersensitizes photographic silver halide emulsions containing methine dyes of the type employed herein. Particularly good results are obtained with dihydroxy substituted reducing agents. Typical dihydroxy compounds which can be employed in the practice of this invention are selected from the group consisting of the benzenes, gamma-lactones, pyronimides, tetronimides, furans and pyrroles, which contain at least two hydroxyl groups.
- 55 Typical useful dihydroxy substituted compounds which can be utilized include hydroquinone, resorcinol, pyrocatechol, 3-methylpyrocatechol, toluehydroquinone, naphthalenediols, etc.;  $\gamma$ -lactones such as ascorbic acid, isoascorbic acid, etc.; 3-hydroxy tetroni-



## 4-hydroxy-6-methyl-1,3,3a,7-tetraazaindene

As noted above, azaindenes function as supersensitizer in emulsions containing various methine dyes. In some emulsions, the azaindene is advantageously used in combination with reducing agent, or preferably sulfonated organic compound supersensitizer, to produce emulsions having the best overall characteristics in terms of inherent emulsion speed, sensitized speed, low fog and storage stability.

According to the invention, one or more of the sulfonated organic compounds or one or more of the azaindenes or one or more of the reducing agents, and one or more of the methine dyes, are added separately or together to light-sensitive photographic silver halide emulsions to supersensitize the emulsions. Particularly good results are frequently obtained when both sulfonated organic compound and reducing agent are employed. In some emulsions, excellent results are obtained with the combination of an azaindene with a sulfonated organic compound supersensitizer. In other instances, it is desirable to supersensitize emulsions with methine dye and sulfonated organic compound, reducing agent and azaindene. The dyes most effectively supersensitized with the compounds described above are the cyanines, particularly the carbocyanine, dicarbocyanine and tricarbocyanine dyes. The enamine tricarbocyanine dyes described herein, such as those of Formula II above, are particularly effective when used with supersensitizer.

The optimum concentration of methine dye and supersensitizer can be determined in a manner well known to those skilled in the art by measuring the sensitivity of test portions of the same emulsion, each portion containing a different concentration of dye and supersensitizer or mixture of supersensitizers. As a general guideline, good results are obtained with about 100 to 2,000 mg dye per mole of silver and about 25 to 2,000 mg and preferably 50 to 1,000 mg per mole of silver of the sulfonated organic supersensitizer.

The silver halide emulsions described herein can be unwashed or washed to remove soluble salts. In the latter case the soluble salts can be removed by chilling, setting and leaching or the emulsion can be coagulation washed, e.g., by the procedures described in Hewitson et al U.S. Pat. No. 2,618,556; Yutzy et al. U.S. Pat. No. 2,614,928; Yackel U.S. Pat. No. 2,565,418; Hart et al. U.S. Pat. No. 3,241,969; and Waller et al. U.S. Pat. No. 2,489,341.

The noble metal and sulfur sensitizers can be added to the emulsion by conventional procedures, such as those described by Smith et al. in U.S. Pat. No. 2,448,060 issued Aug. 31, 1948. Generally, the sensitizers are added at the completion of Ostwald ripening and prior to final digestion.

The silver halide emulsions of this invention can contain speed increasing compounds such as polyalkylene glycols, cationic surface active agents and thioethers or combinations of these as described in Piper U.S. Pat. No. 2,886,437; Chechak U.S. Pat. No. 3,046,134; Carroll et al. U.S. Pat. No. 2,944,900; and Goffe U.S. Pat. No. 3,294,540.

Silver halide emulsions of this invention can be protected against the production of fog and can be stabilized against loss of sensitivity during keeping. Suitable antifoggants and stabilizers, which can be used alone or in combination, include the thiazolium salts described in Staud U.S. Pat. No. 2,131,038 and Allen U.S. Pat.

No. 2,694,716; the azaindenes described in Piper U.S. Pat. No. 2,886,437 and Heimbach U.S. Pat. No. 2,444,605; the mercury salts described in Allen U.S. Pat. No. 2,728,663; the urazoles described in Anderson

5 U.S. Pat. No. 3,287,135; the sulfocatechols described in Kennard U.S. Pat. No. 3,236,652; the oximes described in Carroll et al. British Pat. No. 623,448; nitron; nitroindazoles; the mercaptotetrazoles described in Kendall et al. U.S. Pat. No. 2,403,927, Kennard et al.

10 U.S. Pat. No. 3,266,897 and Luckey et al. U.S. Pat. No. 3,397,987; the polyvalent metal salts described in Jones U.S. Pat. No. 2,839,405; the thiuronium salts described in Herz U.S. Pat. No. 3,220,839; and the palladium, platinum and gold salts described in Trivelli U.S. Pat. No. 2,556,263 and Damschroder U.S. Pat. No. 2,597,915.

Photographic elements including emulsions prepared in accordance with this invention can contain incorporated developing agents such as hydroquinones, catechols, aminophenols, 3-pyrazolidones, ascorbic acid and its derivatives, reductones and phenylenediamines, or combinations of developing agents. The developing agents can be in a silver halide emulsion and/or in another suitable location in the photographic element.

20 25 The developing agents can be added from suitable solvents or in the form of dispersions as described in Yackel U.S. Pat. No. 2,592,368 and Dunn et al. French Pat. No. 1,505,778.

30 Silver halide grains sensitized in accordance with the invention can be dispersed in colloids that can be hardened by various organic or inorganic hardeners, alone or in combination, such as the aldehydes, and blocked aldehydes, ketones, carboxylic and carbonic acid derivatives, sulfonate esters, sulfonyl halides and vinyl sulfones, active halogen compounds, epoxy compounds, aziridines, active olefins, isocyanates, carbodiimides, mixed function hardeners and polymeric hardeners such as oxidized polysaccharides, e.g., dialdehyde

35 40 starch, oxyguargum etc.

Photographic emulsions sensitized in accordance with this invention can contain various colloids alone or in combination as vehicles or binding agents. Suitable hydrophilic materials include both naturally-occurring substances such as proteins, for example, gelatin, gelatin derivatives, cellulose derivatives, polysaccharides such as dextran, gum arabic and the like; and synthetic polymeric substances such as water soluble polyvinyl compounds, e.g., poly(vinyl-pyrrolidone) acrylamide polymers or other synthetic polymeric compounds such as dispersed vinyl compounds in latex form, and particularly those which increase the dimensional stability of the photographic materials. Suitable synthetic polymers include those described, for example, in U.S. Pat. No. 3,142,568 of Nottorf, issued July 28, 1964; 3,193,386 of White, issued July 6, 1965; 3,062,674 of Houck, Smith and Yudelson, issued Nov. 6, 1962; 3,220,844 of Houck, Smith and Yudelson, issued Nov. 30, 1965; Ream and Fowler 3,287,289, issued Nov. 22, 1966; and Dykstra U.S. Pat. No.

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 91

Emulsions supersensitized in accordance with this invention can be used in photographic elements which contain antistatic or conducting layers, such as layers that comprise soluble salts, e.g., chlorides, nitrates, etc., evaporated metal layers, ionic polymers such as those described in Minsk U.S. Pat. No. 2,861,056 and 3,206,312 or insoluble inorganic salts such as those described in Trevoy U.S. Pat. No. 3,428,451.

Photographic emulsions containing the supersensitizing combinations of the invention can be coated on a wide variety of supports. Typical supports include cellulose nitrate film, cellulose ester film, poly(vinyl acetate) film, polystyrene film, poly(ethylene terephthalate) film, polycarbonate film and related films or resinous materials, as well as glass, paper, metal and the like. Typically, a flexible support is employed, especially a paper support, which can be partially acetylated or coated with baryta and/or an alpha-olefin polymer, particularly a polymer of an alpha-olefin containing two to 10 carbon atoms such as polyethylene polypropylene, ethylenebutene copolymers and the like.

Sensitized emulsions of the invention can contain plasticizers and lubricants such as polyalcohols, e.g., glycerin and diols of the type described in Milton U.S. Pat. No. 2,960,404; fatty acids or esters such as those described in Robijns U.S. Pat. No. 2,588,765 and Duane U.S. Pat. No. 3,121,060; and silicone resins such as those described in DuPont British Pat. No. 955,061.

The photographic emulsions sensitized as described herein can contain surfactants such as saponin, anionic compounds such as the alkyl aryl sulfonates described in Baldsiefen U.S. Pat. No. 2,600,831 and amphoteric compounds such as those described in Ben-Ezra U.S. Pat. No. 3,133,816.

Photographic elements containing emulsion layers sensitized as described herein can contain matting agents such as starch, titanium dioxide, zinc oxide, silica, polymeric beads including beads of the type described in Jolley et al. U.S. Pat. No. 2,992,101 and Lynn U.S. Pat. No. 2,701,245.

Sensitized silver halide emulsions of the invention can be utilized in photographic elements which contain brightening agents including stilbene, triazine, oxazole and coumarin brightening agents. Water soluble brightening agents can be used such as those described in Albers et al. German Pat. No. 972,067 and McFall et al. U.S. Pat. No. 2,933,390 or dispersions of brighteners can be used such as those described in Jansen German Pat. No. 1,150,274 and Oetiker et al. U.S. Pat. No. 3,406,070.

Photographic elements containing emulsion layers sensitized by the invention can be used in photographic elements which contain light absorbing materials and filter dyes such as those described in Sawdey U.S. Pat. No. 3,253,921; Gaspar U.S. Pat. No. 2,274,782; Carroll et al. U.S. Pat. No. 2,527,583 and Van Campen U.S. Pat. No. 2,956,879. If desired, the dyes can be mordanted, for example, as described in Milton and Jones U.S. Pat. No. 3,282,699.

The sensitizing dyes (and other emulsion addenda) can be added to the photographic emulsions from water solutions or suitable organic solvent solutions, for example with the procedure described in Collins et al. U.S. Pat. No. 2,912,343; Owens et al. U.S. Pat. No. 3,342,605; Audran U.S. Pat. No. 2,996,287 or Johnson et al. U.S. Pat. No. 3,425,835. The dyes can be dis-

solved separately or together, and the separate or combined solutions can be added to a silver halide emulsion, or a silver halide emulsion layer can be bathed in the solution of dye or dyes.

Photographic emulsions of this invention can be coated by various coating procedures including dip coating, air knife coating, curtain coating, or extrusion coating using hoppers of the type described in Beguin U.S. Pat. No. 2,681,294. If desired, two or more layers 10 may be coated simultaneously by the procedures described in Russell U.S. Pat. No. 2,761,791 and Wynn British Pat. No. 837,095.

Emulsions sensitized as described herein are useful in colloid transfer processes such as described in Yackel 15 et al. U.S. Pat. No. 2,716,059; silver salt diffusion transfer processes such as described in Rott U.S. Pat. No. 2,352,014, Land U.S. Pat. No. 2,543,181, Yackel U.S. Pat. No. 3,020,155 and Land U.S. Pat. No. 2,861,885; color image transfer processes such as described in 20 Rogers U.S. Pat. No. 3,087,817; 3,185,567; and 2,983,606; Weyerts U.S. Pat. No. 3,253,915, Whitmore et al. U.S. Pat. No. 3,227,550; 3,227,551 and 3,227,552; and Land U.S. Pat. No. 3,415,644; 3,415,645; 3,415,646; and imbibition transfer processes as described in Minsk U.S. Pat. No. 2,882,156.

Silver halide emulsions containing the sensitizing combinations of this invention can be used in elements designed for color photography, for example, elements containing color-forming couplers such as those described in Frolich et al. U.S. Pat. No. 2,376,679; Vittum et al. U.S. Pat. No. 2,322,027; Fierke et al. U.S. Pat. No. 2,801,171; Godowsky U.S. Pat. No. 2,698,794; Barr et al. U.S. Pat. No. 3,227,554 and Graham U.S. Pat. No. 3,046,129; or elements to be developed in solutions containing color-forming couplers such as those described in Mannes and Godowsky U.S. Pat. No. 2,252,718; Carroll et al. U.S. Pat. No. 2,592,243 and Schwan U.S. Pat. No. 2,950,970. Exposed photographic emulsions of this invention can be processed by various methods including processing in 35 alkaline solutions containing conventional developing agents such as hydroquinones, catechols, aminophenols, 3-pyrazolidones, phenylenediamines, ascorbic acid derivatives, hydroxylamines, hydrazines and the like; web processing such as described in Tregillus et al. U.S. Pat. No. 3,179,517; stabilization processing as described in Yackel et al. "Stabilization Processing of Films and Papers," *PSA Journal*, Vol. 16B, Aug. 1950; monobath processing as described in Levy "Combined 40 Development and Fixation of Photographic Images with Monobaths," *Phot. Sci. and Eng.*, Vol. 2, No. 3, October, 1958, and Barnes et al. U.S. Pat. No. 3,392,019. If desired, the photographic emulsions of this invention can be processed in hardening developers such as those described in Allen et al. U.S. Pat. No. 3,232,761; in roller transport processors such as those described in Russell U.S. Pat. No. 3,025,779; or by surface application processing as described in Example 3 45 of Kitze U.S. Pat. No. 3,418,132.

The silver halide emulsions sensitized by this invention can be used for making lithographic printing plates such as by the colloid transfer of undeveloped and unhardened areas of an exposed and developed emulsion to a suitable support as described in Clark et al. U.S. Pat. No. 2,763,553; to provide a relief image as described in Woodward U.S. Pat. No. 3,402,045 or Spencer U.S. Pat. No. 3,053,658; to prepare a relief printing

plate as described in Baxter et al. U.S. Pat. No. 3,271,150.

The following examples are included for a further understanding of the invention.

### EXAMPLES 1-8

A set of examples are prepared with four variables in order to illustrate optimum conditions of noble metal and sulfur sensitization of a very fine grain gelatino silver iodobromide (2.5 mole percent iodide) Lippmann emulsion of 0.05  $\mu\text{m}$  grain size. The four variables are (1) level of noble metal sensitization, (2) level of sulfur sensitization, (3) length of time of the chemical sensitization at 65°C, and (4) the level of Dye A with which the emulsion was spectrally sensitized before coating (see structure and name below). Each emulsion is exposed for 10 seconds to a tungsten 500W light source in an Eastman 1B Sensitometer and developed for 4 minutes in Kodak D-19 developer. The coatings are made at approximately 250 mg silver and 600 mg gelatin per square foot on a cellulose acetate support. The results are shown in Table I below.

32

Dye A — Anhydro-3,9-diethyl-5,5'-dimethoxy-3'-(3-sulfopropyl)thiacarbocyanine hydroxide, the red sensitizer used in the examples above.

### EXAMPLE 9

A series of gelatino silver iodobononimide Lippmann emulsions with varying iodide content from 0 to 18.8 mole percent is prepared. The grain size decreases as the iodide content increases. The emulsions are treated in three ways (A) given no further chemical sensitization, (B) chemically sensitized with 176 mg. sodium thiosulfate (23 mg. sulfur) plus 88 mg. potassium tetrachlorate (42 mg. gold) in the range 0 to 10 minutes at 65° C, and (C) chemically sensitized with 30 mg. sodium thiosulfate (3.9 mg. sulfur) plus 300 mg. potassium tetrachloraurate (144 mg. gold) in the range 0 to 10 minutes at 65° C. (Little change is noted within the 0 to 10 minutes time range.) All are coated with 300 mg. of Dye B per mole of silver. The results of photographic tests (conducted as in Examples 1-8) are given in Table II. The above concentrations are given in mg. per mole of silver.

TABLE I

| Example | Noble metal sensitizer (added as $\text{KAuCl}_4$ , mg./per mole Ag) | Sulfur sensitizer (added as $\text{Na}_2\text{S}_2\text{O}_3$ , mg./per mole Ag) | Time of sensitization at $66^\circ\text{C}$ . (min.) | Dye A, mg./per mole Ag | Relative speed | Fog |
|---------|----------------------------------------------------------------------|----------------------------------------------------------------------------------|------------------------------------------------------|------------------------|----------------|-----|
| 1       |                                                                      |                                                                                  | 0                                                    | 0                      | 7.8            | .04 |
| 2       | 25                                                                   | 6.5                                                                              | 20'                                                  |                        | 0              | .08 |
| 3       | 25                                                                   | 6.5                                                                              | 20'                                                  | 1,450                  | 100.0          | .04 |
| 4       | 150                                                                  | 6.5                                                                              | 20'                                                  | 1,450                  | 363.0          | .14 |
| 5       | 75                                                                   | 2.6                                                                              | 40'                                                  | 850                    | 324.0          | .08 |
| 6       | 75                                                                   | 2.6                                                                              | 10'                                                  | 850                    | 259.0          | .08 |
| 7       | 75                                                                   | 16                                                                               | 10'                                                  | 850                    | 126.0          | .04 |
| 8       | 25                                                                   | 6.5                                                                              | 20'                                                  | 500                    | 85.0           | .04 |

Example 1 shows the sensitivity of the primitive emulsion without chemical or spectral sensitization. Example 2 shows a marked decrease in speed upon gold and sulfur sensitization at levels in a range customarily used in the art. Upon spectral sensitization (Example 3), a notable speed increase is observed. In Example 4 a substantially higher level of gold sensitization compared with Example 3 gives a relative speed increase from 100 to 363, accompanied by a small increase in fog. An intermediate but still high level of gold sensitization is indicated in Examples 5 and 6 with lower levels of sulfur sensitization and dye. The relative speeds of these emulsions are high but not as high as in Example 4. Example 7 shows that an increase in sulfur sensitization actually causes a decrease in speed when compared to Example 6. The higher the gold level, the greater the speed. The speed generally varies inversely with the sulfur and the dye levels. Example 8 compared with Example 3 shows little change in speed when a lower level of dye was used. However, the speed drops substantially when the dye is omitted.



TABLE II  
Relative Speed by Chemical

| Emulsion<br>Mole % I | Average<br>Grain Size<br>( $\mu$ m) | Relative Speed by Chemical<br>Sensitization Method |    |     |
|----------------------|-------------------------------------|----------------------------------------------------|----|-----|
|                      |                                     | A                                                  | B  | C   |
| 0                    | 0.052                               | 14                                                 | 71 | 178 |
| 4.7                  | 0.043                               | 16                                                 | 23 | 170 |
| 9.4                  | 0.040                               | 12                                                 | 17 | 126 |
| 18.8                 | 0.034                               | 10                                                 | 13 | 100 |

\*The relative speeds are based on the same scale as Table I.

The data show that the speed effects of the high gold sensitization C persist throughout a wide range of iodide content of the silver iodobromide emulsion. Much smaller speed gains are obtained from the high sulfur and lower gold sensitization (Treatment B). Although some speed loss is noted in going to higher iodide content, the bulk of the effect is attributable to the decreasing grain size of the emulsion. Results generally similar to those in Table II are obtained when the noble metal sensitizer is an equivalent amount of gold, platinum or palladium added, e.g., in the form of potassium iodoaurate, auric trichloride, potassium aurithiocyanate, a compound of the formula:



ammonium chloropalladate, sodium chloroplatinate, ammonium chlororuthenate or ammonium chloroiodate. Also, generally similar results to those in Table II are obtained when the sulfur sensitizer is added in an equivalent amount of a sulfur sensitizer other than sodium thiosulfate, such as thiourea, thiosinamine. Likewise, results generally similar to those in Table II are obtained when the various methine dyes referred to herein are substituted for dye B.

A series of Lippman gelatin silver bromoiodide (2.5 mole percent of the halide being iodide) emulsions are prepared and coated on a cellulose acetate support at a concentration of 250 mg. silver per square foot and 1041 mg. gelatin per square foot. The emulsions are chemically sensitized with potassium tetrachloroaurate and sodium thiosulfate, with 10 minute digestion at 65° C after addition of the chemical sensitizers. Various dyes, identified in Table T below, are added to the emulsions, which have the grain size and contain the concentration of chemical sensitizer given in the following tables. Supersensitizer "A" is 4,4'-bis[4,6-bis-o-chloroanilino-s-triazin-2-yl] amino]-2,2'-stilbenedisulfonic acid, sodium salt in amounts of 1,000 mg. per mole of silver and Supersensitizer B (ascorbic acid) in amounts of 500 mg. per mole of silver are added as is described in the tables below. Each emulsion is exposed and developed as described in Examples 1-9 above, except that an exposure is made through Kodak Wratten Filters 35 and 2B to record the blue (365 line) exposure.

TABLE III

Silver halide grain size 0.09; 300 mg. potassium tetrachloroaurate per mole of silver (about 150 mg. gold per mole of silver) and 30 mg. sodium thiosulfate (about 4 mg. sulfur per mole of silver):

| Dye     | Mg. dye per mole of silver | Super-sensitizer | Relative blue speed | Sensitization | Fogmaximum |    |
|---------|----------------------------|------------------|---------------------|---------------|------------|----|
| Control | —                          | —                | 8.0                 | 0.07          | —          | 40 |
| 1       | 450                        | —                | 200                 | 0.08          | 535        |    |
| 2       | 569                        | —                | 60                  | 0.06          | 495        |    |
| 3       | 818                        | A                | 182                 | 0.16          | 525        |    |
| 4       | 847                        | —                | 55                  | 0.06          | 495        |    |
| 5       | 510                        | —                | 200                 | 0.06          | 490        |    |
| Control | —                          | —                | 6.5                 | 0.08          | —          | 45 |
| 1       | 600                        | —                | 200                 | 0.08          | 540        |    |
| 6       | 515                        | A                | 117                 | 0.10          | 540        |    |
| 7       | 810                        | A                | 174                 | 0.09          | 540        |    |
| 8       | 843                        | —                | 158                 | 0.08          | 565        |    |
| 9       | 562                        | —                | 148                 | 0.08          | 565        |    |
| 10      | 548                        | —                | 105                 | 0.11          | 550        |    |
| 11      | 444                        | —                | 174                 | 0.08          | 535        |    |
| 12      | 556                        | A                | 14                  | 0.06          | —          | 50 |
| 13      | 663                        | A                | 200                 | 0.08          | 525        |    |
| 14      | 541                        | A                | 129                 | 0.09          | 525        |    |
| 15      | 569                        | A                | 158                 | 0.08          | 570        | 2  |
| 16      | 366                        | A                | 105                 | 0.08          | 540        |    |
| 17      | 125                        | —                | —                   | —             | —          |    |
| Control | —                          | —                | 100                 | 0.12          | Pan        | 3  |
| 18      | 125                        | A+B              | 302                 | 0.12          | Pan        | 55 |
| 19      | 450                        | —                | 6.2                 | 0.08          | —          | 4  |
| 20      | 543                        | —                | 200                 | 0.07          | 540        |    |
| 21      | 343                        | A+B              | 135                 | 0.08          | 525        |    |
| 22      | 645                        | —                | 117                 | 0.08          | 535        | 5  |
| 23      | 690                        | —                | 83                  | 0.06          | 525        |    |
| 24      | 540                        | —                | 71                  | 0.09          | 545        | 6  |
| 25      | 562                        | —                | 234                 | 0.07          | 535        |    |
| Control | —                          | —                | 174                 | 0.06          | 535        | 7  |
| 1       | 450                        | —                | 5.9                 | 0.06          | —          |    |
| 21      | 794                        | —                | 200                 | 0.06          | 540        | 8  |
| 22      | 820                        | —                | 100                 | 0.07          | 515        |    |
| 23      | 480                        | A                | 58                  | 0.08          | 525        | 65 |
| 24      | 714                        | —                | 43                  | 0.08          | 525        | 9  |
| 9       | 411                        | A                | 129                 | 0.08          | 525        |    |
| 25      | 246                        | A                | 110                 | 0.10          | 545        | 10 |
|         |                            |                  | 71                  | 0.06          | 530        |    |

|    | 10  | 26  | Control | 296 | 437 | A   | 245  | 0.08 | 535 |
|----|-----|-----|---------|-----|-----|-----|------|------|-----|
| 17 | —   | —   | —       | —   | —   | —   | 2.2  | 0.02 | —   |
| 17 | 300 | —   | 300     | —   | —   | 93  | 0.12 | 715  |     |
| 16 | 300 | A+B | 300     | A+B | 170 | 170 | 0.12 | 640  |     |
| 27 | 300 | A+B | 300     | A+B | 155 | 155 | 0.22 | 720  |     |
| 28 | 287 | A+B | 287     | A+B | 170 | 170 | 0.20 | 720  |     |
| 29 | 333 | A+B | 333     | A+B | 162 | 162 | 0.14 | 710  |     |
| 30 | 318 | A+B | 318     | A+B | 170 | 170 | 0.20 | 710  |     |
| 31 | 265 | A+B | 265     | A+B | 170 | 170 | 0.24 | 700  |     |
| 32 | 189 | —   | 189     | —   | 200 | 200 | 0.08 | 565  |     |

TABLE IV

Silver halide grain size 0.09; 200 mg. potassium tetrachloroaurate per mole of silver (about 100 mg. gold per mole of silver) and 20 mg. sodium thiosulfate per mole of silver (about 2.6 mg. sulfur per mole of silver):

| Dye     | Mg. dye per mole of silver | Super-sensitizer | Relative blue speed | Sensitization |
|---------|----------------------------|------------------|---------------------|---------------|
| Control | —                          | —                | 4.0                 | 0.06          |
| 17      | 300                        | A+B              | 174                 | 0.08          |
| 32      | 500                        | —                | 200                 | 0.06          |

TABLE V

Silver halide grain size 0.05 micron; 320 mg. potassium tetrachloroaurate per mole of silver (about 160 mg. gold per mole of silver) and 32 mg. sodium thiosulfate per mole of silver (about 4 mg. sulfur per mole of silver):

| Dye     | Mg. dye per mole of silver | Super-sensitizer | Relative blue speed | Sensitization |
|---------|----------------------------|------------------|---------------------|---------------|
| Control | —                          | —                | 1.3                 | 0.06          |
| 32      | 574                        | —                | 200                 | 0.09          |
| 37      | 558                        | —                | 78                  | 0.09          |
| 38      | 629                        | —                | 86                  | 0.08          |
| 39      | 1926                       | —                | 37                  | 0.07          |
| Control | —                          | —                | 1.4                 | 0.06          |
| 32      | 574                        | —                | 200                 | 0.10          |
| 32      | 765                        | —                | 209                 | 0.12          |
| 40      | 671                        | —                | 209                 | 0.10          |
| 40      | 895                        | —                | 200                 | 0.12          |

TABLE T

| Dye No. | Dye Name                                                                                             |
|---------|------------------------------------------------------------------------------------------------------|
| 1       | 3-Allyl-5-[5,5-dimethyl-3-(3-pyrrolin-1-yl)-2-cyclohexenylidene]rhodanine                            |
| 2       | 5-[5,6-Dichloro-1,3-diethyl-2-benzimidazolinylidene]ethylidene]-1-ethyl-2-thiobarbituric acid        |
| 3       | 3-Ethyl-5-[(3-ethyl-2-benzothiazolinylidene)-ethylidene]-2-(2-thiazolyl)imino-4-imidazolidinone      |
| 4       | 1-(2-Diethylaminoethyl)-5-[(3-ethyl-2-benzoxazolinylidene)ethylidene]-3-phenyl-2-thiobarbituric acid |
| 5       | 3,6,3'-8-Di-(trimethylene)triazolinocarbocyanine perchlorate                                         |
| 6       | 3-Ethyl-2-[4-(3-pyrrolin-1-yl)-1,3-pentadienyl]benzothiazolium perchlorate                           |
| 7       | 5,6-Dichloro-1,3'-diethyl-3-[2-(1-pyrrolidinyl)-ethyl]benzimidazoloxacarbocyanine iodide             |
| 8       | 1,1',3,3'-Tetraethyl-5,5'-bis(trifluoromethyl)-benzimidazoloxacarbocyanine iodide                    |
| 9       | 2-[4-(1-Piperidyl)-1,3-butadienyl]-β-naphthothiazole ethiodide                                       |
| 10      | 3-Ethyl-5-(3-methyl-2-thiazolinylidene-ethylidene)-1-phenyl-2-thiohydantoin                          |

- 11 1-[4-(4-morpholyl)- $\Delta^{1,3}$ -butadienyl]benzothiazole ethiodide  
 12 3-Ethyl-5-[3-methyl-2-thiazolidinylidene]ethylidene]-1-(2-morpholinoethyl)-2-thiohydantoin  
 13 1-(2-Diethylaminoethyl)-5-[3-methyl-2-thiazolidinylidene]ethylidene]-3-phenyl-2-thiohydantoin  
 14 3-Ethyl-5-[3-(4-sulfobutyl-2-(3H)-benzoazolylidene]ethylidene]rhodanine  
 15 3-Ethyl-5-[ $\gamma$ -(1-piperidyl)allylidene]rhodanine  
 16 3-Ethyl-2-[2-[2,3,4,4a,5,6-hexahydro-7-(1-pyrrolidinyl)-1-naphthyl]vinyl]  
 17 {benzoazolium 2,3,4,4a,5,6  
 18 3,3'-Diethyl-6,6'-dimethoxythiadicarbocyanine p-toluenesulfonate  
 19 3-Ethyl-2-[4-(1,2,5,6-tetrahydro-1-pyridyl)-3,4-trimethylene-1,3-butadienyl]benzoazolium perchlorate  
 20 2-[6-Ethoxycarbonyl-3-(1-pyrrolidinyl)-2-cyclohexenylidene]methyl-3-ethylbenzothiazolium perchlorate  
 21 2,3'-Bis(3,3-diethoxypropyl)-9-ethyl-5,5'-diphenyloxacarbocyanine bromide  
 22 2,2'-Diethyloxacarbocyanine iodide  
 23 2,2'-Diethyl-8-methyloxacarbocyanine iodide  
 4,4'-Dichloro-2,2',8-triethyloxacarbocyanine iodide  
 24 3,3'-Diethyl-4,4-dimethyl-4',5'-benzoazolinothiacarbocyanine fluoroborate  
 25 3-Ethyl-5-[3-ethyl-2-oxazolidinylidene]ethylidene]rhodanine  
 26 4-[(-Ethyl-2(1- $\beta$ -naphthothiazolylidene)isopropylidene]-3-methyl-1-(p-sulfonyl)-5-pyrazolone  
 27 3,3'-Diethyl-10,12-ethylene-11-(4-phenyl-1-piperazinyl)oxatricarbocyanine perchlorate  
 28 3,3'-Diethyl-10,12-ethylene-11-(1,2,3,4-tetrahydro-2-isquinolyl)oxatricarbocyanine perchlorate  
 29 (3,3'-Diethyl-10,12-ethylene-11-[4-(3-phenylpropyl)piperidino]thiatricarbocyanine perchlorate  
 30 3,3'-Diethyl-10,12-ethylene-11-[4-(3-phenylpropyl)piperidino]oxatricarbocyanine perchlorate  
 31 3,3'-Diethyl-10,12-ethylene-11-(1,2,5,6-tetrahydro-1-pyridyl)oxatricarbocyanine perchlorate  
 32 3-Ethyl-5-[2-(3-pyrroline-1-yl)-1-cyclopentenylmethylene]rhodanine  
 33 3-Ethyl-5-[1-indolinyl]-5,5-dimethyl-2-cyclohexen-1-ylidene]ethylidene rhodanine  
 34 Anhydro-3-methyl-9-(2-pyrrolyl)-3'-(3-sulfopropyl)-4,5;4',5'-dibenzothiacarbocyanine hydroxide  
 35 3,3'-Diethyl-7,7'-dimethoxythiadicarbocyanine iodide  
 36 2-[(1-Carboxymethyl-4-oxo-3-phenyl-2-thioxo-5-imidazolidinylidene)ethylidene]-3-ethyl-1-phenyl-5-[(1,3,3-trimethylene-2-indolinylidene)ethylidene]-4-imidazolidinone  
 37 5-[2-(1-Azetidinyl)-1-cyclopentenylmethylene]-3-ethylrhodanine  
 38 3-Ethyl-5-[3-ethyl-2-(3)-benzoazolylidene]isopropylidene rhodanine  
 39 Anhydro-1-allyl-5-chloro-3'-ethyl-5'-methoxy-3-(3-sulfopropyl)benzimidazolo-oxacarbocyanine hydroxide  
 40 3-Carboxymethyl-5-[2-(3-pyrrolin-1-yl)-1-cyclopentenylmethylene]rhodanine, sodium salt

Silver halide emulsions sensitized as described herein are particularly useful in microelectronic manufacturing, e.g., solid state circuit production, and in the production of holograms. These materials are described, for example, in Kodak Data Book P-9, *Kodak Films and Plates for Science and Industry*, published by the Eastman Kodak Co., 1967. Emulsions employed for such purposes advantageously contain a high concentration of at least one removable and substantially photographically inert light absorbing dye, as described in Stevens British Pat. No. 1,139,062. Since these materials are generally exposed to a mercury vapor source which emits in the blue region of the spectrum at 405

nm and 436 nm and in the green region at 547 nm, it is desirable that the silver halide exhibit high sensitivity to all three line exposures. The use of absorbing dyes to reduce image spread and produce images of exceptionally high sharpness reduces the speed and contrast of these elements as described in Kodak British Pat. No. 1,139,062. It is, therefore, desirable to increase either or both blue and green speeds. The combination of a benzothiazolinylidene-thioxazolidinedione blue sensitizer with the oxathiazolocarbocyanine green sensitizer described in Stevens British Pat. No. 1,139,062 gives increased blue sensitivity with little or no change in green sensitivity. An increased concentration of the green sensitizer (above that which normally causes desensitization) gives an increase in green sensitivity without a substantial loss of contrast.

A particularly useful sensitizer is 3-ethyl-5-(3-ethyl-2-benzothiazolinylidene)-2-thio-2,4-oxazolidine-dione, which can be used effectively at concentrations of about 600 to 800 mg. per mole of silver. An effective green sensitizer is 3,3'-diethyl-4'-methyloxathiazolocarbocyanine iodide, which can be used effectively at 400, and preferably at 800 mg. per mole of silver. The combination of such sensitizers provides good blue and green speeds when the emulsion is exposed to a mercury vapor illuminant. Also highly useful is the dye 3-ethyl-5-[2-(3-pyrrolin-1-yl)-1-cyclopentenylmethylene]rhodanine

30



40 which gives high contrast and a substantial speed increase on exposure to both blue and green radiation when employed in emulsions sensitized in accordance with the invention.

45 Good results are also obtained with cyanine, merocyanine or hemicyanine dyes having a tertiary aminoalkyl group substituted on a heterocyclic nitrogen atom of the dye, such as 6-chloro-3,3'-diethyl-1-(2-morpholinoethyl)benzimidazolo-oxacarbocyanine iodide. Other useful dyes and dye combinations include anhydro-9-ethyl-3,3'-di(3-sulfopropyl)-4,5;4',5'-dibenzothiacarbocyanine hydroxide, sodium salt; anhydro-3-ethyl-9-methyl-3'-(3-sulfobutyl)thiacarbocyanine hydroxide; anhydro-1'-ethyl-3-(3-sulfobutyl)thia-2'-cyanine hydroxide; 3-ethyl-5-(3-ethyl-2-benzothiazolinylidene)-2-thio-2,4-oxazolidinedione; 3,3'-diethyl-4'-methyloxathiazolocarbocyanine iodide; anhydro-3,9-diethyl-5,5'-dimethoxy-3'-(3-sulfopropyl)-thiacarbocyanine hydroxide; or, anhydro-9-ethyl-5,5'-dimethoxy-3,3'-bis(3-sulfopropyl)thiacarbocyanine hydroxide, sodium salt.

55 The following dyes provide highly useful results: 3-ethyl-2-[4,6-neopentylene-6-(4-methyl-1-piperazinyl)-1,3,5-hexatrienyl]benzothiazolium iodide, 3-ethyl-2-[6-(4-ethoxycarbonyl-1-piperazinyl)-4,6-neopentylene-1,3,5-hexatrienyl]-benzothiazolium iodide, and 3-ethyl-2-[6-(4-ethoxycarbonyl-1-piperazinyl)-4,6-neopentylene-1,3,5-hexatrienyl]ben-

zoxazolium iodide. These dyes can be used alone, or in combination with other dyes, such as 3,3'-diethyl-6,6'-dimethoxythiadi carbocyanine p-toluenesulfonate. These dyes, whether used alone or in combination with other dyes, can be supersensitized, e.g., with a polynuclear aromatic compound containing at least one sulfo group (such as 4,4'-bis[4,6-bis-o-chloroanilino-s-triazin-2-yl amino]-2,2'-stilbenedisulfonic acid, sodium salt), and/or a reducing agent (such as ascorbic acid).

The invention has been described in detail with particular reference to preferred embodiments thereof, but, it will be understood that variations and modifications can be effected within the spirit and scope of the invention.

We claim:

1. A photographic silver halide emulsion comprising light-sensitive silver halide grains having an average grain size up to about 0.2 micron; said silver halide grains being sensitized with the combination of a gold sensitizer, at a concentration of about 50 to 200 milligrams 2 gold per mole of silver, and a sulfur sensitizer at a weight ratio of sulfur to gold of from 1:15 to 1:75; and, said silver halide being spectrally sensitized with at least one dye having one of the following formulas:



wherein Z, Z<sub>1</sub>, Z<sub>4</sub> and Z<sub>5</sub> each represents the non-metallic atoms necessary to complete a heterocyclic nucleus containing from 5 to 6 atoms; each L represents a methine linkage; d, n, c, e and g each represents an integer of from one to two; p and f each represents an integer of from one to three; m represents an integer of from one to five; R<sub>1</sub>, R<sub>2</sub>, R<sub>7</sub> and R<sub>8</sub> each represents an alkyl group or an aryl group; X and X<sub>2</sub> each represents an acid anion; Q, Q<sub>1</sub> and Q<sub>2</sub> each represents the non-metallic atoms required to complete a nitrogen-containing heterocyclic nucleus containing from 5 to 6 atoms in the heterocyclic ring; D represents an enamine group selected from a 2,3,4,4a,5,6-hexahydro-7-(1-pyrrolidinyl)-1-naphthyl group; a 2,6,7,7a-tetrahydro-5-(1-pyrrolidinyl)-3-indenyl group, a 3-(1-pyrrolidinyl)-2-norbornen-2yl group; a 3-(1-pyrrolidinyl)-2-indenyl group or a group having one of the following formulas:



10

15 and D<sup>1</sup> represents a group having the following formula:



25. 2. A photographic silver halide emulsion as defined in claim 6 wherein the light-sensitive silver halide grains have an average grain size of from about 0.02 to about 0.09 micron.

3. A photographic silver halide emulsion comprising  
30 light-sensitive silver halide grains having an average  
grain size up to about 0.1 micron; said silver halide  
grains being sensitized with the combination of a gold  
sensitizer, at a concentration of about 50 to 200 milli-  
grams gold per mole of silver, and a sulfur sensitizer at  
35 a weight ratio of sulfur to gold of from 1:15 to 1:75;  
and, said silver halide being spectrally sensitized with  
a methine dye having one of the following formulas:



50 wherein  $e$  and  $g$  each represents a positive integer of from one to two;  $f$  represents a positive integer of from one to three;  $L$  represents a methine linkage;  $R_8$  represents an alkyl group or an aryl group;  $Z_5$  represents the non-metallic atoms necessary to complete a heterocyclic nucleus containing from 5 to 6 atoms in the heterocyclic ring;  $Q_1$  and  $Q_2$  each represents the non-metallic atoms required to complete a heterocyclic nucleus containing from 5 to 6 atoms in the heterocyclic ring;  $X_2$  represents an acid anion;  $D$  represents a group having one of the following formulas:



6





and, D<sup>1</sup> represents a group having the following formula:



4. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3-allyl-5-[5,5-dimethyl-3-(3-pyrrolin-1-yl)-2-cyclohexenylidene]rhodanine.

5. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3,6;3,8-di-(trimethylene)thiazolino carbocyanine salt.

6. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3-ethyl-5-[3-methyl-2-thiazolidinylidene)ethylidene]-1-(2-morpholinoethyl)-2-thiohydantoin, said dye being supersensitized with 4,4'-bis[4,6-bis-o-chloroanilino-s-triazin-2-yl]amino]-2,2'-stilbene-disulfonic acid, disodium salt.

7. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3-allyl-5-[5,5-dimethyl-3-(3-pyrrolin-1-yl)-2-cyclohexenylidene]rhodanine; 3-ethyl-2-{2-[2,3,4,4a,5,6-hexahydro-7-(1-pyrrolidinyl)-1-

naphthyl]vinyl}benzoxazolium salt; and, 3,3'-diethyl-6,6'-dimethoxythiadicarbocyanine salt, said dyes being supersensitized with 4,4'-bis[4,6-bis-o-chloroanilino-s-triazin-2-yl]amino]-2,2'-stilbene-disulfonic acid, disodium salt and ascorbic acid.

8. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3-ethyl-5-[2-(3-pyrrolin-1-yl)-1-cyclopentenylmethylene]rhodanine.

9. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3-carboxymethyl-5-[2-(3-pyrrolin-1-yl)-1-cyclopentenylmethylene]rhodanine, sodium salt.

10. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3-ethyl-2-{2-[2,3,4,4a%,4-hexahydro-7-(1-pyrrolidinyl)-1-naphthyl]vinyl}benzoxazolium salt.

11. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 5,6-dichloro-1,3'-diethyl-3-[2-(1-pyrrolidinyl)ethyl]benzimidazolo-oxacarbocyanine salt.

12. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3-ethyl-5-(3-methyl-2-thiazolinylidene-ethylidene)-1-phenyl-2-thiohydantoin.

13. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50; said silver halide being spectrally sensitized with 3,3'-diethyl-6,6'-dimethoxythiadicarbocyanine salt.

14. A photographic gelatin silver halide emulsion in which the silver halide grains have an average grain size

of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50, said silver halide being spectrally sensitized with anhydro-3,9-diethyl-5,5'-dimethoxy-3'-(3-sulfopropyl)thiocarbocyanine hydroxide.

15. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50, said silver halide being spectrally sensitized with anhydro-9-ethyl-5,5'-dimethoxy-3,3'-bis(3-sulfopropyl)thiocarbocyanine hydroxide, sodium salt.

16. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50, said silver halide being spectrally sensitized with 6-chloro-3,3'-diethyl-1-(2-morpholinoethyl)benzimidazolooxacarbocyanine salt.

17. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50, said silver halide being spectrally sensitized with 3-ethyl-2-[4,6-neopentylene-6-(4-methyl-1-

piperazinyl)-1,3,5-hexatrienyl]benzothiazolium salt together with 3,3'-diethyl-6,6'-dimethoxythiadcarbocyanine salt.

18. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50, said silver halide being spectrally sensitized with 3-ethyl-2-[6-(4-ethoxycarbonyl-1-piperazinyl)-4,6-neopentylene-1,3,5-hexatrienyl]benzothiazolium salt together with 3,3'-diethyl-6,6'-dimethoxythiadcarbocyanine salt.

19. A photographic gelatin silver halide emulsion in which the silver halide grains have an average grain size of from about 0.02 to about 0.09 micron; said grains being sensitized with the combination of potassium tetrachloroaurate, at a concentration of about 125 to 175 mg. gold per mole of silver, together with sodium thiosulfate at a weight ratio of sulfur to gold of from 1:30 to 1:50, said silver halide being spectrally sensitized with 3-ethyl-2-[6-(4-ethoxycarbonyl-1-piperazinyl)-4,6-neopentylene-1,3,5-hexatrienyl]benzoxazolium salt together with 3,3'-diethyl-6,6'-dimethoxythiadcarbocyanine salt.

20. In a light sensitive photographic silver halide emulsion comprising silver halide grains having a grain size up to about 0.2 micron, which grains are spectrally sensitized with a methine dye and chemically sensitized with a gold sensitizer and a sulfur sensitizer, the improvement wherein said gold sensitizer is present at a concentration of at least 50 mg. per mole of silver, and said sulfur sensitizer is present at a ratio of sulfur to gold of from 1:15 to 1:75.

\* \* \* \* \*